

# United States Patent [19]

Shirai et al.

[11] Patent Number: 4,792,509

[45] Date of Patent: \* Dec. 20, 1988

[54] LIGHT RECEIVING MEMBER FOR USE IN ELECTROPHOTOGRAPHY

[75] Inventors: Shigeru Shirai, Shiga; Keishi Saitoh, Nagahama; Takayoshi Arai, Nagahama; Minoru Kato, Nagahama; Yasushi Fujioka, Nagahama, all of Japan

[73] Assignee: Canon Kabushiki Kaisha, Tokyo, Japan

[\*] Notice: The portion of the term of this patent subsequent to Apr. 19, 2005 has been disclaimed.

[21] Appl. No.: 10,001

[22] Filed: Feb. 2, 1987

[30] Foreign Application Priority Data

Feb. 4, 1986 [JP] Japan ..... 61-22546  
Feb. 5, 1986 [JP] Japan ..... 61-24604

[51] Int. Cl.<sup>4</sup> ..... G03G 5/085

[52] U.S. Cl. ..... 430/64; 430/66;  
430/84; 430/95

[58] Field of Search ..... 430/65, 64, 57, 58,  
430/84, 66, 95

[56] References Cited

U.S. PATENT DOCUMENTS

4,678,731 7/1987 Yoshizawa ..... 430/954

Primary Examiner—John L. Goodrow

Attorney, Agent, or Firm—Fitzpatrick, Cella, Harper & Scinto

[57] ABSTRACT

There is provided an improved light receiving member for use in electrophotography comprising a substrate for electrophotography and a light receiving layer constituted by a charge injection inhibition layer formed of a polycrystal material containing silicon atoms as the main constituent atoms and an element for controlling the conductivity which functions to prevent a charge from being injected from the side of the substrate, a photoconductive layer formed of an amorphous material containing silicon atoms as the main constituent atoms and a surface layer formed of an amorphous material containing silicon atoms, carbon atoms and hydrogen atoms, the amount of the hydrogen atoms contained in the surface layer being in the range from 41 to 70 atomic %. The light receiving layer may have a contact layer and/or an absorption layer of light having a long wavelength.

17 Claims, 14 Drawing Sheets

FIG. 1(A)



FIG. 1 (B)



FIG. 1 (C)



FIG. 1 (D)



FIG. 2



FIG. 5



FIG. 3



FIG. 6



FIG. 4



FIG. 7



FIG. 8



FIG. 9



FIG. 10



FIG. 11



FIG. 12



FIG. 13



FIG. 14



FIG. 15



FIG. 16



FIG. 17



FIG. 18



FIG. 19



FIG. 20(A)



FIG. 20(B)



FIG. 20(C)



FIG. 21



FIG. 22



FIG. 23



FIG. 24



FIG. 25



FIG. 26



FIG. 27



FIG. 28



**LIGHT RECEIVING MEMBER FOR USE IN ELECTROPHOTOGRAPHY**

**FIELD OF THE INVENTION**

This invention relates to an improved light receiving member for use in electrophotography which is sensitive to electromagnetic waves such as light (which herein means in a broader sense those lights such as ultra-violet rays, visible rays, infrared rays, X-rays and  $\gamma$ -rays).

**BACKGROUND OF THE INVENTION**

For the photoconductive material to constitute a light receiving layer in a light receiving member for use in electrophotography, it is required to be highly sensitive, to have a high SN ratio [photocurrent ( $I_p$ )/dark current ( $I_d$ )], to have absorption spectrum characteristics suited for the spectrum characteristics of an electromagnetic wave to be irradiated, to be quickly responsive and to have a desired dark resistance. It is also required to be not harmful to living things as well as man upon the use.

Especially, in the case where it is the light receiving member to be applied in an electrophotographic machine for use in office, causing no pollution is indeed important.

From these standpoints, the public attention has been focused on light receiving members comprising amorphous materials containing silicon atoms (hereinafter referred to as "a-Si"), for example, as disclosed in *Offenlegungsschriften* Nos. 2746967 and 2855718 which disclose use of the light receiving member as an image-forming member in electrophotography.

For the conventional light receiving members comprising a-Si materials, there have been made improvements in their optical, electric and photoconductive characteristics such as dark resistance, photosensitivity, and photoresponsiveness, use-environmental characteristics, economic stability and durability.

However, there are still left subjects to make further improvements in their characteristics in the synthesis situation in order to make such light receiving member practically usable.

For example, in the case where such conventional light receiving member is employed in the light receiving member for use in electrophotography with aiming at heightening the photosensitivity and dark resistance, there are often observed a residual voltage on the conventional light receiving member upon the use, and when it is repeatedly used for a long period of time, fatigues due to the repeated use will be accumulated to cause the so-called ghost phenomena inviting residual images.

Further, in the preparation of the light receiving layer of the conventional light receiving member for use in electrophotography using an a-Si material, hydrogen atoms, halogen atoms such as fluorine atoms or chlorine atoms, elements for controlling the electrical conduction type such as boron atoms or phosphorus atoms, or other kinds of atoms for improving the characteristics are selectively incorporated in the light receiving layer.

However, the resulting light receiving layer sometime becomes accompanied with defects on the electrical characteristics, photoconductive characteristics

and/or breakdown voltage according to the way of the incorporation of said constituents to be employed.

That is, in the case of using the light receiving member having such light receiving layer, the life of a photo-carrier generated in the layer with the irradiation of light is not sufficient, the inhibition of a charge injection from the side of the substrate in a dark layer region is not sufficiently carried out, and image defects likely due to a local breakdown phenomenon which is so-called "white oval marks on half-tone copies" or other image defects likely due to abrasion upon using a blade for the cleaning which is so-called "white line" are apt to appear on the transferred images on a paper sheet.

Further, in the case where the above light receiving member is used in a much moist atmosphere, or in the case where after being placed in that atmosphere it is used, the so-called "image flow" sometimes appears on the transferred images on a paper sheet.

In consequence, it is necessitated not only to make a further improvement in an a-Si material itself but also to establish such a light receiving member not to invite any of the foregoing problems.

**SUMMARY OF THE INVENTION**

The object of this invention is to provide a light receiving member for use in electrophotography which has a light receiving layer free from the foregoing problems and capable of satisfying various kind of requirements in electrophotography.

That is, the main object of this invention is to provide a light receiving member for use in electrophotography which has a light receiving layer comprising a layer formed of a-Si and a layer formed of a polycrystal material containing silicon atoms (hereinafter referred to as "poly-Si"), that electrical, optical and photoconductive properties are always substantially stable scarcely depending on the working circumstances, and that is excellent against optical fatigue, causes no degradation upon repeating use, excellent in durability and moisture-proofness and exhibits no or scarce residual voltage.

Another object of this invention is to provide a light receiving member for use in electrophotography which has a light receiving layer comprising a layer formed of a-Si and a layer formed of poly-Si, which is excellent in the close bondability with a substrate on which the layer is disposed or between the laminated layers, dense and stable in view of the structural arrangement and is of high quality.

A further object of this invention is to provide a light receiving member for use in electrophotography which has a light receiving layer comprising a layer formed of a-Si and a layer formed of poly-Si, which exhibits a sufficient charge-maintaining function in the electrification process of forming electrostatic latent images and excellent electrophotographic characteristics when it is used in electrophotographic method.

A still further object of this invention is to provide a light receiving member for use in electrophotography which has a light receiving layer comprising a layer formed of a-Si and a layer formed of poly-Si, which invites neither an image defect nor an image flow on the resulting visible images on a paper sheet upon repeated use in a long period of time and which gives highly resolved visible images with clearer half-tone which are highly dense and quality.

Other object of this invention is to provide a light receiving member for use in electrophotography which has a light receiving layer comprising a layer formed of

a-Si and a layer formed of poly-Si, which has a high photosensitivity, high S/N ratio and high electrical voltage withstanding property.

In order to overcome the foregoing problems on the conventional light receiving member for use in electrophotography and attaining the above-mentioned objects, the present inventors have made various studies while focusing on its surface layer and other constituent layer. As a result, the present inventors have found that when the surface layer is formed of an amorphous material containing silicon atoms, carbon atoms and hydrogen atoms and the content of the hydrogen atoms is controlled to be in the range between 41 and 70 atomic %, and that when at least one of other constituent layers except the surface layer is formed of a polycrystal material containing silicon atoms, those problems on the conventional light receiving member for use in electrophotography can be satisfactorily eliminated and the abovementioned objects can be effectively attained.

Accordingly, this invention is to provide a light receiving member for use in electrophotography basically comprising a substrate usable for electrophotography, a light receiving layer comprising a charge injection inhibition layer formed of a polycrystal material containing silicon atoms as the main constituent atoms and an element for controlling the conductivity, a photoconductive layer formed of an amorphous material containing silicon atoms as the main constituent atoms and at least one kind selected from hydrogen atoms and halogen atoms [hereinafter referred to as "A-Si(H,X)"], and a surface layer having a free surface being formed of an amorphous material containing silicon atoms, carbon atoms and hydrogen atoms (hereinafter referred to as "A-Si:C:H") in which the amount of the hydrogen atoms to be contained is ranging from 41 to 70 atomic %.

It is possible for the light receiving member according to this invention to have an absorption layer for light of long wavelength (hereinafter referred to as "IR layer"), which is formed of an amorphous material or a polycrystal material containing silicon atoms and germanium atoms, and if necessary, at least either hydrogen atoms or halogen atoms [hereinafter referred to as "A-SiGe (H,X)" or "poly-SiGe(H,X)"], between the substrate and the charge injection inhibition layer.

It is also possible for the light receiving member according to this invention to have a contact layer, which is formed of an amorphous material or a polycrystal material containing silicon atoms as the main constituent atoms and at least one kind selected from nitrogen atoms, oxygen atoms and carbon atoms [hereinafter referred to as "A-Si(N,O,C)" or "poly-Si(N,O,C)"], between the substrate and the IR layer or between the substrate and the charge injection inhibition layer.

And the above-mentioned photoconductive layer may contain one or more kinds selected from oxygen atoms, nitrogen atoms, and an element for controlling the conductivity as the layer constituent atoms.

The above-mentioned charge injection inhibition layer may contain hydrogen atoms and/or halogen atoms, and, further, in case where necessary, at least one kind selected from nitrogen atoms, oxygen atoms and carbon atoms as the layer constituent atoms.

The above-mentioned IR layer may contain one or more kinds selected from nitrogen atoms, oxygen atoms, carbon atoms, and an element for controlling the conductivity as the layer constituent atoms.

The light receiving member having the above-mentioned light receiving layer for use in electrophotography according to this invention is free from the foregoing problems on the conventional light receiving members for use in electrophotography, has a wealth of practically applicable excellent electric, optical and photoconductive characteristics and is accompanied with an excellent durability and satisfactory use environmental characteristics.

Particularly, the light receiving member for use in electrophotography according to this invention has substantially stable electric characteristics without depending on the working circumstances, maintains a high photosensitivity and a high S/N ratio and does not invite any undesirable influence due to residual voltage even when it is repeatedly used for along period of time. In addition, it has sufficient moisture resistant and optical fatigue resistance, and cause neither degradation upon repeating use nor any defect on breakdown voltage.

Because of this, according to the light receiving member for use in electrophotography of this invention, even upon repeated use for a long period of time, highly resolved visible images with clearer half tone which are highly dense and quality are stably obtained.

#### BRIEF DESCRIPTION OF THE DRAWINGS

FIG. 1(A) through FIG. 1(D) are schematic views illustrating the typical layer constitution of a representative light receiving member for use in electrophotography according to this invention;

FIG. 2 through FIG. 7 are views illustrating the thicknesswise distribution of germanium atoms in the IR layer;

FIG. 8 through FIG. 12 are views illustrating the thicknesswise distribution of the group III atoms or the group V atoms in the charge injection inhibition layer;

FIG. 13 through FIG. 19 are views illustrating the thicknesswise distribution of at least one kind selected from nitrogen atoms, oxygen atoms, and carbon atoms in the charge injection inhibition layer;

FIG. 20(A) through FIG. 20(C) are schematic views for examples of the shape at the surface of the substrate in the light receiving member for use in electrophotography according to this invention;

FIG. 21 is a schematic view for a preferred example of the light receiving member for use in electrophotography according to this invention which has a light receiving layer as shown in FIG. 1(C) formed on the substrate having a preferred surface;

FIGS. 22 through 23 are schematic explanatory views of a preferred method for preparing the substrate having the preferred surface used in the light receiving member shown in FIG. 21;

FIG. 24 is a schematic explanatory view of a fabrication apparatus for preparing the light receiving member for use in electrophotography according to this invention;

FIG. 25 and FIG. 26 are schematic views respectively illustrating the shape of the surface of the substrate in the light receiving member in Examples 9 and 23, and Examples 10 and 24;

FIG. 27 is a view illustrating the thicknesswise distribution of boron atoms and oxygen atoms in the charge injection inhibition layer in Example 2; and

FIG. 28 is a view illustrating the thicknesswise distribution of boron atoms and oxygen atoms in the charge

injection inhibition layer and germanium atoms in IR layer in Example 12.

#### DETAILED DESCRIPTION OF THE INVENTION

Representative embodiments of the light receiving member for use in electrophotography according to this invention will now be explained more specifically referring to the drawings. The description is not intended to limit the scope of this invention.

Representative light receiving members for use in electrophotography according to this invention are as shown in FIG. 1(A) through FIG. 1(D), in which are shown light receiving layer 100, substrate 101, charge injection inhibition layer 102, photoconductive layer 103, surface layer 104, free surface 105, IR layer 106, and contact layer 107.

FIG. 1(A) is a schematic view illustrating a typical representative layer constitution of this invention, in which is shown the light receiving member comprising the substrate 101 and the light receiving layer 100 constituted by the charge injection inhibition layer 102, the photoconductive layer 103 and the surface layer 104.

FIG. 1(B) is a schematic view illustrating another representative layer constitution of this invention, in which is shown the light receiving member comprising the substrate 101 and the light receiving layer 100 constituted by the IR layer 106, the charge injection inhibition layer 102, the photoconductive layer 103 and the surface layer 104.

FIG. 1(C) is a schematic view illustrating another representative layer constitution of this invention, in which is shown the light receiving member comprising the substrate 101 and the light receiving layer 100 constituted by the contact layer 107, the IR layer 106, the charge injection inhibition layer 102, the photoconductive layer 103 and the surface layer 104.

FIG. 1(D) is a schematic view illustrating another representative layer constitution of this invention, in which is shown the light receiving member comprising the substrate 101 and the light receiving layer constituted by the contact layer 107, the charge injection inhibition layer 102, the photoconductive layer 103 and the surface layer 104.

Now, explanation will be made for the substrate and each constituent layer in the light receiving member of this invention.

#### Substrate 101

The substrate 101 for use in this invention may either be electroconductive or insulative. The electroconductive support can include, for example, metals such as NiCr, stainless steels, Al, Cr, Mo, Au, Nb, Ta, V, Ti, Pt and Pb or the alloys thereof.

The electrically insulative support can include, for example, films or sheets of synthetic resins such as poly-ester, polyethylene, polycarbonate, cellulose acetate, polypropylene, polyvinyl chloride, polyvinylidene chloride, polystyrene, and polyamide, glass, ceramic and paper. It is preferred that the electrically insulative substrate is applied with electroconductive treatment to at least one of the surfaces thereof and disposed with a light receiving layer on the thus treated surface.

In the case of glass, for instance, electroconductivity is applied by disposing, at the surface thereof, a thin film made of NiCr, Al, Cr, Mo, Au, Ir, Nb, Ta, V, Ti, Pt, Pd, In<sub>2</sub>O<sub>3</sub>, SnO<sub>2</sub>, ITO (In<sub>2</sub>O<sub>3</sub> + SnO<sub>2</sub>), etc. In the case of the synthetic resin film such as a polyester film, the electro-

conductivity is provided to the surface by disposing a thin film of metal such as NiCr, Al, Ag, Pv, Zn, Ni, Au, Cr, Mo, Ir, Nb, Ta, V, Ti and Pt by means of vacuum deposition, electron beam vapor deposition, sputtering, etc., or applying lamination with the metal to the surface. The substrate may be of any configuration such as cylindrical, belt-like or plate-like shape, which can be properly determined depending on the application uses. For instance, in the case of using the light receiving member shown in FIG. 1 in continuous high speed reproduction, it is desirably configurated into an endless belt or cylindrical form.

The thickness of the support member is properly determined so that the light receiving member as desired can be formed.

In the case where flexibility is required for the light receiving member, it can be made as thin as possible within a range capable of sufficiently providing the function as the substrate. However, the thickness is usually greater than 10  $\mu\text{m}$  in view of the fabrication and handling or mechanical strength of the substrate.

And, it is possible for the surface of the substrate to be uneven in order to eliminate occurrence of defective images caused by a so-called interference fringe pattern being apt to appear in the formed images in the case where the image formation is carried out using coherent monochromatic light such as laser beams.

In that case, the uneven surface shape of the substrate can be formed by the grinding work with means of an appropriate cutting tool, for example, having a V-form bite.

That is, said cutting tool is firstly fixed to the predetermined position of milling machine or lathe, then, for example, a cylindrical substrate is moved regularly in the predetermined direction while being rotated in accordance with the predetermined program to thereby obtain a surface-treated cylindrical substrate of a surface having irregularities in reverse V-form with a desirably pitch and depth.

The irregularities thus formed at the surface of the cylindrical substrate form a helical structure along the center axis of the cylindrical substrate. The helical structure making the reverse V-form irregularities of the surface of the cylindrical substrate may be double or treble. Or otherwise, it may be of a cross-helical structure.

Further, the irregularities at the surface of the cylindrical substrate may be composed of said helical structure and a delay line formed along the center axis of the cylindrical substrate. The cross-sectional form of the convex of the irregularity formed at the substrate surface is in a reverse V-form in order to attain controlled unevenness of the layer thickness in the minute column for each layer to be formed and secure desired close bondability and electric contact between the substrate and the layer formed directly thereon.

And it is desirable for the reverse V-form to be an equilateral triangle, right-angled triangle or inequilateral triangle. Among these triangle forms, equilateral triangle form and right-angled triangle form are most preferred.

Each dimension of the irregularities to be formed at the substrate surface under the controlled conditions is properly determined having a due regard on the following points.

That is, firstly, a layer composed of, for example, a-Si(H,X) or poly-Si(H,X) to constitute a light receiving layer is structurally sensitive to the surface state of the

layer to be formed and the layer quality is apt to largely change in accordance with the surface state.

Therefore, it is necessary for the dimension of the irregularity to be formed at the substrate surface to be determined not to invite any decrease in the layer quality.

Secondly, should there exist extreme irregularities on the free surface of the light receiving layer, cleaning in the cleaning process after the formation of visible images becomes difficult to sufficiently carry out. In addition, in the case of carrying out the cleaning with a blade, the blade will be soon damaged.

From the viewpoints of avoiding the problems in the layer formation and the electrophotographic processes, and from the conditions to prevent occurrence of the problems due to interference fringe patterns, the pitch of the irregularity to be formed at the substrate surface is preferably 0.3 to 500  $\mu\text{m}$ , more preferably 1.0 to 200  $\mu\text{m}$ , and most preferably, 5.0 to 50  $\mu\text{m}$ .

As for the maximum depth of the irregularity, it is preferably 0.1 to 5.0  $\mu\text{m}$ , more preferably 0.3 to 3.0  $\mu\text{m}$ , and, most preferably, 0.6 to 2.0  $\mu\text{m}$ .

And when the pitch and the depth of the irregularity lie respectively in the above-mentioned range, the inclination of the slope of the dent (or the linear convex) of the irregularity is preferably 1° to 20°, more preferably 3° to 15°, and, most preferably, 4° to 10°.

Further, as for the maximum figure of a thickness difference based on the ununiformity in the layer thickness of each layer to be formed on such substrate surface, in the meaning within the same pitch, it is preferably 0.1 to 2.0  $\mu\text{m}$ , more preferably 0.1 to 1.5  $\mu\text{m}$ , and, most preferably, 0.2  $\mu\text{m}$  to 1.0  $\mu\text{m}$ .

In alternative, the irregularity at the substrate surface may be composed of a plurality of fine spherical dimples which are more effective in eliminating the occurrence of defective images caused by the interference fringe patterns especially in the case of using coherent monochromatic light such as laser beams.

In that case, the scale of each of the irregularities composed of a plurality of fine spherical dimples is smaller than the resolving power required for the light receiving member for use in electrophotography.

A typical method of forming the irregularities composed of a plurality of fine spherical dimples at the substrate surface will be hereunder explained referring to FIGS. 22 and 23.

FIG. 22 is a schematic view for a typical example of the shape at the surface of the substrate in the light receiving member for use in electrophotography according to this invention, in which a portion of the uneven shape is enlarged. In FIG. 22, are shown a support 2201, a support surface 2202, a rigid true sphere 2203, and a spherical dimple 2204.

FIG. 22 also shows an example of the preferred methods of preparing the surface shape as mentioned above. That is, the rigid true sphere 2203 is caused to fall gravitationally from a position at a predetermined height above the substrate surface 2202 and collide against the substrate surface 2202 to thereby form the spherical dimple 2204. A plurality of fine spherical dimples 2204 each substantially of an identical radius of curvature  $R$  and of an identical width  $D$  can be formed to the substrate surface 2202 by causing a plurality of rigid true spheres 2203 substantially of an identical diameter  $R'$  to fall from identical height  $h$  simultaneously or sequentially.

FIG. 23 shows a typical embodiment of a substrate formed with the uneven shape composed of a plurality of spherical dimples at the surface as described above.

In the embodiment shown in FIG. 23, a plurality of dimples 2304, 2304 . . . substantially of an identical radius of curvature and substantially of an identical width are formed while being closely overlapped with each other thereby forming an uneven shape regularly by causing to fall a plurality of spheres 2303, 2303, . . . regularly and substantially from an identical height to different positions at the surface 2302 of the support 2301. In this case, it is naturally required for forming the dimples 2304, 2304 . . . overlapped with each other that the spheres 2303, 2303 . . . are gravitationally dropped such that the times of collision of the respective spheres 2303 to the support 2302 and displaced from each other.

By the way, the radius of curvature  $R$  and the width  $D$  of the uneven shape formed by the spherical dimples at the substrate surface of the light receiving member for use in electrophotography according to this invention constitute an important factor for effectively attaining the advantageous effect of preventing occurrence of the interference fringe in the light receiving member for use in electrophotography according to this invention. The present inventors carried out various experiments and, as a result, found the following facts.

That is, if the radius of curvature  $R$  and the width  $D$  satisfy the following equation:

$$D/R \geq 0.035$$

0.5 or more Newton rings due to the sharing interference are present in each of the dimples. Further, if they satisfy the following equation:

$$D/R \geq 0.055$$

one or more Newton rings due to the sharing interference are present in each of the dimples.

From the foregoing, it is preferred that the ratio  $D/R$  is greater than 0.035 and, preferably, greater than 0.055 for dispersing the interference fringes resulted throughout the light receiving member in each of the dimples thereby preventing occurrence of the interference fringe in the light receiving member.

Further, it is desired that the width  $D$  of the unevenness formed by the scraped dimple is about 500  $\mu\text{m}$  at the maximum, preferably, less than 200  $\mu\text{m}$  and, more preferably less than 100  $\mu\text{m}$ .

FIG. 21 is a schematic view illustrating a representative embodiment of the light receiving member in which is shown the light receiving member comprising the above-mentioned substrate 2101 and the light receiving layer 100 constituted by contact layer 2107, IR layer 2106, charge injection inhibition layer 2102, photoconductive layer 2103, and surface layer 2104 having free surface 2105.

#### Contact Layer 107 (or 2107)

The contact layer 107 (or 2107) of this invention is formed of an amorphous material or a polycrystal material containing silicon atoms, at least one kind selected from nitrogen atoms, oxygen atoms and carbon atoms, and if necessary, hydrogen atoms or/and halogen atoms.

Further, the contact layer may contain an element for controlling conductivity.

The main object of disposing the contact layer in the light receiving member of this invention is to enhance the bondability between the substrate and the charge injection inhibition layer or between the substrate and the IR layer. And, when the element for controlling the conductivity is incorporated in the contact layer, the transportation of a charge between the substrate and the charge injection inhibition layer is effectively improved.

For incorporating various atoms in the contact layer, that is, at least one kind selected from nitrogen atoms, oxygen atoms and carbon atoms; elements for controlling the conductivity in case where necessary; they may be distributed either uniformly in the entire layer region or unevenly in the direction toward its layer thickness.

In the light receiving member of this invention, the amount of nitrogen atoms, oxygen atoms, or carbon atoms to be incorporated in the contact layer is properly determined according to use purposes.

It is preferably  $5 \times 10^{-4}$  to  $7 \times 10$  atomic %, more preferably  $1 \times 10^{-3}$  to  $5 \times 10$  atomic %, and, most preferably,  $2 \times 10^{-3}$  to  $3 \times 10$  atomic %.

For the thickness of the contact layer, it is properly determined having a due regard to its bondability, charge transporting efficiency, and also to its productivity.

It is preferably  $1 \times 10^{-2}$  to  $1 \times 10 \mu\text{m}$ , and most preferably,  $2 \times 10^{-2}$  to  $5 \mu\text{m}$ .

As for the hydrogen atoms and halogen atoms to be optionally incorporated in the contact layer, the amount of hydrogen atoms or halogen atoms, or the sum of the amount of hydrogen atoms and the amount of halogen atoms in the contact layer is preferably  $1 \times 10^{-1}$  to  $7 \times 10$  atomic %, more preferably  $5 \times 10^{-1}$  to  $5 \times 10$  atomic %, and, most preferably, 1 to  $3 \times 10$  atomic %.

#### IR Layer 106 (or 2106)

In the light receiving member for use in electrophotography of this invention, the IR layer is formed of either A-SiGe(H,X) or poly-SiGe(H,X).

As for the germanium atoms to be contained in the IR layer, they may be distributed uniformly in its entire layer region or unevenly in the direction toward the layer thickness of its entire layer region.

However, in any case, it is necessary for the germanium atoms to be distributed uniformly in the direction parallel to the surface of the substrate in order to provide the uniformness of the characteristics to be brought out.

[Herein or hereinafter, the uniform distribution means that the distribution of germanium atoms in the layer is uniform both in the direction parallel to the surface of the substrate and in the thickness direction. The uneven distribution means that the distribution of germanium atoms in the layer is uniform in the direction parallel to the surface of the substrate but is uneven in the thickness direction.]

That is, in the case where the germanium atoms are contained unevenly in the direction toward the layer thickness of its entire layer region, the germanium atoms are incorporated so as to be in the state that these atoms are more largely distributed in the layer region near the substrate than in the layer apart from the substrate (namely in the layer region near the free surface of the light receiving layer) or in the state opposite to the above state.

In preferred embodiments, the germanium atoms are contained unevenly in the direction toward the layer thickness of the entire layer region of the IR layer.

In one of the preferred embodiments, the germanium atoms are contained in such state that the distributing concentration of these atoms is changed in the way of being decreased from the layer region near the substrate toward the layer region near the charge injection inhibition layer. In this case, the affinity between the IR layer and the charge injection inhibition becomes excellent. And, as later detailed, when the distributing concentration of the germanium atoms is made significantly large in the layer region adjacent to the substrate, the IR layer becomes to substantially and completely absorb the light of long wavelength that can be hardly absorbed by the photoconductive layer in the case of using a semiconductor laser as the light source. As a result, the occurrence of the interference caused by the light reflection from the surface of the substrate can be effectively prevented.

Explanation will be made to the typical embodiments of the distribution of germanium atoms to be contained unevenly in the direction toward the layer thickness of the IR layer while referring to FIGS. 2 through 7 showing the distribution of germanium atoms. However, this invention is no way limited only to these embodiments.

In FIGS. 2 through 7, the abscissa represent the distribution concentration C of germanium atoms and the ordinate represents the thickness of the IR layer; and  $t_B$  represents the extreme position of the IR layer containing germanium atoms is formed from the  $t_B$  side toward the  $t_T$  side.

FIG. 2 shows the first typical example of the thicknesswise distribution of the germanium atoms in the IR layer. In this example, germanium atoms are distributed such that the concentration C remains constant at a value  $C_1$  in the range from position  $t_B$  (at which the IR layer comes into contact with the substrate) to position  $t_1$ , and the concentration C gradually and continuously decreases from  $C_2$  in the range from position  $t_1$  to position  $t_7$ , where the concentration of the germanium atoms is  $C_3$ .

In the example shown in FIG. 3, the distribution concentration C of the germanium atoms contained in the IR layer is such that concentration  $C_4$  at position  $t_B$  continuously decreases to concentration  $C_5$  at position  $t_T$ .

In the example shown in FIG. 4, the distribution concentration C of the germanium atoms is such that the concentration  $C_6$  remains constant in the range from position  $t_B$  and position  $t_2$  and it gradually and continuously decreases in the range from position  $t_2$  and position  $t_T$ . The concentration at position  $t_T$  is substantially zero. ("Substantially zero" means that the concentration is lower than the detectable limit.)

In the example shown in FIG. 5, the distribution concentration C of the germanium atoms is such that concentration  $C_8$  gradually and continuously decreases in the range from position  $t_B$  and position  $t_T$ , at which it is substantially zero.

In the example shown in FIG. 6, the distribution concentration C of the germanium atoms is such that concentration  $C_9$  remains constant in the range from position  $t_B$  to position  $t_3$ , and concentration  $C_9$  linearly decreases to concentration  $C_{10}$  in the range from position  $t_3$  to position  $t_T$ .

In the example shown in FIG. 7, the distribution concentration C of the germanium atoms is such that

concentration  $C_{11}$  linearly decreases in the range from position  $t_B$  to position  $t_7$ , at which the concentration is substantially zero.

Several examples of the thicknesswise distribution of germanium atoms in the IR layer are illustrated in FIGS. 2 through 7. In the light receiving member of this invention, the concentration (C of germanium atoms in the IR layer is preferred to be high at the position adjacent to the substrate and considerably low at the position adjacent to the interface  $t_7$ .

The thicknesswise distribution of germanium atoms contained in the IR layer is such that the maximum concentration  $C_{max}$  of germanium atoms is preferably greater than  $1 \times 10^3$  atomic ppm, more preferably greater than  $5 \times 10^3$  atomic ppm, and most preferably, greater than  $1 \times 10^4$  atomic ppm based on the total amount of silicon atoms and germanium atoms.

For the amount of germanium atoms to be contained in the IR layer, it is properly determined according to desired requirements. However, it is preferably 1 to  $1 \times 10^6$  atomic ppm, more preferably  $10^2$  to  $9.5 \times 10^5$  atomic ppm, and, most preferably,  $5 \times 10^2$  to  $8 \times 10^5$  atomic ppm based on the total amount of silicon atoms and germanium atoms.

Further, the IR layer may contain at least one kind selected from the element for controlling the conductivity, nitrogen atoms, oxygen atoms and carbon atoms.

In that case, its amount is preferably  $1 \times 10^{-2}$  to  $4 \times 10$  atomic %, more preferably  $5 \times 10^{-2}$  to  $3 \times 10$  atomic %, and most preferably  $1 \times 10^{-1}$  to 25 atomic %.

As for the element for controlling the conductivity, so-called impurities in the field of the semiconductor can be mentioned and those usable herein can include atoms belonging to the group III of the periodic table that provide p-type conductivity (hereinafter simply referred to as "group III atoms") or atoms belonging to the group V of the periodic table that provide n-type conductivity (hereinafter simply referred to as "group V atoms"). Specifically, the group III atoms can include B (boron), Al (aluminum), Ga (gallium), In (indium) and Tl (thallium), B and Ga being particularly preferred. The group V atoms can include P (phosphorus), As (arsenic), Sb (antimony), and Bi (bismuth), P and Sb being particularly preferred.

For the amount of the element for controlling the conductivity, it is preferably  $1 \times 10^{-2}$  to  $5 \times 10^5$  atomic ppm, more preferably  $5 \times 10^{-1}$  to  $1 \times 10^4$  atomic ppm, and, most preferably, 1 to  $5 \times 10^3$  atomic ppm.

And as for the thickness of the IR layer, it is preferably 30 Å to 50 µm, more preferably 40 Å to 40 µm, and, most preferably, 50 Å to 30 µm.

#### Charge Injection Inhibition Layer 102 (or 2102)

In the light receiving member for use in electrophotography of this invention, the charge injection inhibition layer is formed of poly-Si(H,X) containing the element for controlling the conductivity uniformly in the entire layer region or largely in the side of the substrate.

And said layer may contain at least one kind selected nitrogen atoms, oxygen atoms and carbon atoms in the state of being distributed uniformly in the entire layer region or partial layer region but largely in the side of the substrate.

Now, the charge injection inhibition layer can be disposed on the substrate, the IR layer, or the contact layer.

The halogen atom (X) to be contained in the charge injection inhibition layer include preferably F (fluorine), Cl (chlorine), Br (bromine), and I (iodine), F and Cl being particularly preferred.

The amount of hydrogen atoms (H), the amount of the hydrogen atoms (X) or the sum of the amounts for the hydrogen atoms and the halogen atoms (H+X) contained in the charge injection inhibition layer is preferably 1 to 40 atomic %, and, most preferably, 5 to 30 atomic %.

As for the element for controlling the conductivity to be contained in said layer, the group III or group V atoms can be used likewise in the case of the above-mentioned IR layer.

Explanation will be made to the typical embodiments for distributing the group III atoms or group V atoms in the direction toward the layer thickness in the charge injection inhibition layer while referring to FIGS. 8-12.

In FIGS. 8 through 12, the abscissa represents the distribution concentration C of the group III atoms or group V atoms and the ordinate represents the thickness of the charge injection inhibition layer; and  $t_B$  represents the extreme position of the layer adjacent to the substrate and  $t_7$  represents the other extreme position of the layer which is away from the substrate.

The charge injection inhibition layer is formed from the  $t_B$  side toward the  $t_7$  side.

FIG. 8 shows the first typical example of the thicknesswise distribution of the group III atoms or group V atoms in the charge injection inhibition layer. In this example, the group III atoms or group V atoms are distributed such that the concentration C remains constant at a value  $C_{12}$  in the range from position  $t_B$  to position  $t_4$ , and the concentration C gradually and continuously decreases from  $C_{13}$  in the range from position  $t_4$  to position  $t_7$ , where the concentration of the group III atoms or group V atoms is  $C_{14}$ .

In the example shown in FIG. 9, the distribution concentration C of the group III atoms or group V atoms contained in the light receiving layer is such that concentration  $C_{15}$  at position  $t_B$  continuously decreases to concentration  $C_{16}$  at position  $t_7$ .

In the example shown in FIG. 10, the distribution concentration C of the group III atoms or group V atoms is such that concentration  $C_{17}$  remains constant in the range from position  $t_B$  to position  $t_3$ , and concentration  $C_{17}$  linearly decreases to concentration  $C_{18}$  in the range from position  $t_5$  to position  $t_7$ .

In the example shown in FIG. 11, the distribution concentration C of the group III atoms or group V atoms is such that concentration  $C_{19}$  remains constant in the range from position  $t_B$  and position  $t_6$  and it linearly decreases from  $C_{20}$  to  $C_{21}$  in the range from position  $t_6$  to position  $t_7$ .

In the example shown in FIG. 12, the distribution concentration C of the group III atoms or group V atoms is such that concentration  $C_{22}$  remains constant in the range from position  $t_B$  and position  $t_7$ .

In the case where the group III atoms or group V atoms are contained in the charge injection inhibition layer in such way that the distribution concentration of the atoms in the direction of the layer thickness is higher in the layer region near the substrate, the thicknesswise distribution of the group III atoms or group V atoms is preferred to be made in the way that the maximum concentration of the group III atoms or group V atoms is controlled to be preferably greater than 50 atomic ppm, more preferably greater than 80 atomic

pmm, and, most preferably, greater than  $10^2$  atomic ppm.

For the amount of the group III atoms or group V atoms to be contained in the charge injection inhibition layer, it is properly determined according to desired requirements. However, it is preferably  $3 \times 10$  to  $5 \times 10^5$  atomic ppm, more preferably  $5 \times 10$  to  $1 \times 10^4$  atomic ppm, and, most preferably,  $1 \times 10^2$  to  $5 \times 10^3$  atomic ppm.

When at least one kind selected from nitrogen atoms, oxygen atoms and carbon atoms is incorporated in the charge injection inhibition layer, not only the mutual contact between the IR layer and the charge injection inhibition layer and the bondability between the charge injection inhibition layer and the photoconductive layer but also the adjustment of band gap for that layer are effectively improved.

Explanation will be made to the typical embodiments for distributing at least one kind selected from nitrogen atoms, oxygen atoms and carbon atoms in the direction toward the layer thickness in the charge injection inhibition layer, with reference to FIGS. 13 through 19.

In FIGS. 13 through 19, the abscissa represents the distribution concentration C of at least one kind selected from nitrogen atoms, oxygen atoms and carbon atoms, and the ordinate represents the thickness of the charge injection inhibition layer; and  $t_B$  represents the extreme position of the layer adjacent to the substrate and  $t_T$  represents the other extreme position of the layer which is away from the substrate. The charge injection inhibition layer is formed from the  $t_B$  side toward the  $t_T$  side.

FIG. 13 shows the first typical example of the thicknesswise distribution of at least one kind selected from nitrogen atoms, oxygen atoms and carbon atoms in the charge injection inhibition layer. In this example, at least one kind selected from nitrogen atoms, oxygen atoms and carbon atoms are distributed such that the concentration C remains constant at a value  $C_{23}$  in the range from position  $t_B$  to position  $t_7$ , and the concentration C gradually and continuously decreases from  $C_{24}$  in the range from position  $t_7$  to position  $t_T$ , where the concentration of at least one kind selected from nitrogen atoms, oxygen atoms, and carbon atoms is  $C_{25}$ .

In the example shown in FIG. 14, the distribution concentration C of at least one kind selected from nitrogen atoms, oxygen atoms, and carbon atoms contained in the charge injection inhibition layer is such that concentration  $C_{26}$  at position  $t_B$  continuously decreases to concentration  $C_{27}$  at position  $t_T$ .

In the example shown in FIG. 15, the distribution concentration C of at least one kind selected from nitrogen atoms, oxygen atoms, and carbon atoms is such that concentration  $C_{28}$  remains constant in the range from position  $t_B$  and position  $t_8$  and it gradually and continuously decreases from position  $t_8$  and becomes substantially zero between  $t_8$  and  $t_T$ .

In the example shown in FIG. 16, the distribution concentration C of at least one kind selected from nitrogen atoms, oxygen atoms and carbon atoms is such that concentration  $C_{30}$  gradually and continuously decreases from position  $t_B$  and becomes substantially zero between  $t_B$  and  $t_T$ .

In the example shown in FIG. 17, the distribution concentration C of at least one kind selected from nitrogen atoms, oxygen atoms and carbon atoms is such that concentration  $C_{31}$  remains constant in the range from position  $t_B$  to position  $t_9$ , and concentration  $C_9$  linearly

decreases to concentration  $C_{32}$  in the range from position  $t_9$  to position  $t_7$ .

In the example shown in FIG. 18, the distribution concentration C of at least one kind selected from nitrogen atoms, oxygen atoms and carbon atoms is such that concentration  $C_{33}$  remains constant in the range from position  $t_B$  and position  $t_{10}$  and it linearly decreases from  $C_{34}$  to  $C_{35}$  in the range from position  $t_{10}$  to position  $t_7$ .

In the example shown in FIG. 19, the distribution concentration C of at least one kind selected from nitrogen atoms, oxygen atoms and carbon atoms is such that concentration  $C_{36}$  remains constant in the range from position  $t_B$  and position  $t_T$ .

In the case where at least one kind selected from nitrogen atoms, oxygen atoms and carbon atoms is contained in the charge injection inhibition layer such that the distribution concentration of these atoms in the layer is higher in the layer region near the substrate, the thicknesswise distribution of at least one kind selected from nitrogen atoms, oxygen atoms and carbon atoms is made in such way that the maximum concentration of at least one kind selected from nitrogen atoms, oxygen atoms and carbon atoms is controlled to be preferably greater than  $5 \times 10^2$  atomic ppm, more preferably, greater than  $8 \times 10^2$  atomic ppm, and, most preferably, greater than  $1 \times 10^3$  atomic ppm.

As for the amount of at least one kind selected from nitrogen atoms, oxygen atoms and carbon atoms is properly determined according to desired requirements. However, it is preferably  $1 \times 10^{-3}$  to 50 atomic %, more preferably,  $2 \times 10^{-3}$  atomic % to 40 atomic %, and, most preferably,  $3 \times 10^{-3}$  to 30 atomic %.

For the thickness of the charge injection inhibition layer, it is preferably  $1 \times 10^{-2}$  to  $10 \mu\text{m}$ , more preferably,  $5 \times 10^{-2}$  to  $8 \mu\text{m}$ , and, most preferably,  $1 \times 10^{-1}$  to  $5 \mu\text{m}$  in the viewpoints of bringing about electrophotographic characteristics and economical effects.

#### Photoconductive Layer 103 (or 2103)

The photoconductive layer 103 (or 2103) is disposed on the substrate 101 (or 2102) as shown in FIG. 1 (or FIG. 21).

The photoconductive layer is formed of an A-Si(H,X) material or an A-Si(H,X)(O,N) material.

The photoconductive layer has the semiconductor characteristics as under mentioned and shows a photoconductivity against irradiated light.

(i) p-type semiconductor characteristics: containing an acceptor only or both the acceptor and a donor in which the relative content of the acceptor is higher;

(ii) p-type semiconductor characteristics: the content of the acceptor (Na) is lower or the relative content of the acceptor is lower in the case (i);

(iii) n-type semiconductor characteristics: containing a donor only or both the donor and an acceptor in which the relative content of the donor is higher;

(iv) n-type semiconductor characteristics: the content of donor (Nd) is lower or the relative content of the acceptor is lower in the case (iii); and

(v) i-type semiconductor characteristics:  $\text{Na} \approx \text{Nd} = 0$  or  $\text{Na} \approx \text{Nd}$ .

In order for the photoconductive layer to be a desirable type selected from the above-mentioned types (i) to (v), it can be carried out by doping a p-type impurity, an n-type impurity or both the impurity with the photoconductive layer to be formed during its forming process while controlling the amount of such impurity.

As the element to be such impurity to be contained in the photoconductive layer, the so-called impurities in the field of the semiconductor can be mentioned, and those usable herein can include atoms belonging to the group III or the periodical table that provide p-type conductivity (hereinafter simply referred to as "group III atom") or atoms belonging to the group V of the periodical table that provide n-type conductivity (hereinafter simply referred to as "group V atom"). Specifically, the group III atoms can include B (boron), Al (aluminum), Ga (gallium), In (indium) and Tl (thallium). The group V atoms can include, for example, P (phosphor), As (arsenic), Sb (antimony) and Bi (bismuth). Among these elements, B, Ga, P and As are particularly preferred.

The amount of the group III atoms or the group V atoms to be contained in the photoconductive layer is preferably  $1 \times 10^{-3}$  to  $3 \times 10^2$  atomic ppm, more preferably,  $5 \times 10^{-3}$  to  $1 \times 10^2$  atomic ppm, and, most preferably,  $1 \times 10^{-2}$  to 50 atomic ppm.

In the photoconductive layer, oxygen atoms or/and nitrogen atoms can be incorporated in the range as long as the characteristics required for that layer is not hindered.

In the case of incorporating oxygen atoms or/and nitrogen atoms in the entire layer region of the photoconductive layer, its dark resistance and close bondability with the substrate are improved.

The amount of oxygen atoms or/and nitrogen atoms to be incorporated in the photoconductive layer is desired to be relatively small not to deteriorate its photoconductivity.

In the case of incorporating nitrogen atoms in the photoconductive layer, its photosensitivity in addition to the above advantages may be improved when nitrogen atoms are contained together with boron atoms therein.

The amount of one kind selected from nitrogen atoms (N), and oxygen atoms (O) or the sum of the amounts for two kinds of these atoms to be contained in the photoconductive layer is preferably  $5 \times 10^{-2}$  to 30 atomic %, more preferably,  $1 \times 10^2$  to 20 atomic %, and, most preferably,  $2 \times 10^{-2}$  to 15 atomic %.

The amount of the hydrogen atoms (H), the amount of the halogen atoms (H) or the sum of the amounts for the hydrogen atoms and the halogen atoms (H+X) to be incorporated in the photoconductive layer is preferably 1 to 40 atomic %, more preferably, 5 to 30 atomic %.

The halogen atom (X) includes, specifically, fluorine, chlorine, bromine and iodine. And among these halogen atoms, fluorine and chlorine and particularly preferred.

The thickness of the photoconductive layer is an important factor in order for the photocarriers generated by the irradiation of light having desired spectrum characteristics to be effectively transported, and it is appropriately determined depending upon the desired purpose.

It is, however, also necessary that the layer thickness be determined in view of relative and organic relationships in accordance with the amounts of the halogen atoms and hydrogen atoms contained in the layer or the characteristics required in the relationship with the thickness of other layer. Further, it should be determined also in economical viewpoints such as productivity or mass productivity. In view of the above, the thickness of the photoconductive layer is preferably 1

to 100  $\mu\text{m}$ , more preferably, 1 to 80  $\mu\text{m}$ , and, most preferably, 2 to 50  $\mu\text{m}$ .

#### Surface Layer 104 (or 2104)

5 The surface layer 104 (or 2104) having the free surface 105 (or 2105) is disposed on the photoconductive layer 103 (or 2103) to attain the objects chiefly of moisture resistance, deterioration resistance upon repeating use, electrical voltage withstanding property, use environmental characteristics and durability for the light receiving member for use in electrophotography according to this invention.

The surface layer is formed of the amorphous material containing silicon atoms as the constituent element 15 which are also contained in the layer constituent amorphous material for the photoconductive layer, so that the chemical stability at the interface between the two layers is sufficiently secured.

Typically the surface layer is formed of an amorphous material containing silicon atoms, carbon atoms, and hydrogen atoms (hereinafter referred to as "A-( $\text{Si}_x\text{C}_{1-x}$ )<sub>y</sub> $\text{H}_{1-y}$ ",  $x > 0$  and  $y < 1$ ).

It is necessary for the surface layer for the light receiving member for use in electrophotography according to this invention to be carefully formed in order for that layer to bring about the characteristics as required.

That is, a material containing silicon atoms (Si), carbon atoms (C) and hydrogen atoms (H) as the constituent elements is structurally extended from a crystalline state to an amorphous state which exhibit electrophysically properties from conductiveness to semiconductiveness and insulativeness, and other properties from photoconductiveness to in photoconductiveness according to the kind of a material.

35 Therefore, in the formation of the surface layer, appropriate layer forming conditions are required to be strictly chosen under which a desired surface layer composed of A- $\text{Si}_x\text{C}_{1-x}$  having the characteristics as required may be effectively formed.

For instance, in the case of disposing the surface layer with aiming chiefly at improvements in its electrical voltage withstanding property, the surface layer composed of A-( $\text{Si}_x\text{C}_{1-x}$ )<sub>y</sub> $\text{H}_{1-y}$  is so formed that it exhibits a significant electrical insulative behavior in use environment.

45 In the case of disposing the surface layer with aiming at improvements in repeating use characteristics and use environmental characteristics, the surface layer composed of A- $\text{Si}_x\text{C}_{1-x}$  is so formed that it has certain sensitivity to irradiated light although the electrical insulative property should be somewhat decreased.

The amount of carbon atoms and the amount of hydrogen atoms respectively to be contained in the surface layer of the light receiving member for use is electrophotography according to this invention are important factors as well as the surface layer forming conditions in order to make the surface layer accompanied with desired characteristics to attain the objects of this invention.

55 The amount of the carbon atoms (C) to be incorporated in the surface layer is preferably  $1 \times 10^{-3}$  to 90 atomic %, and, most preferably, 10 to 80 atomic % respectively to the sum of the amount of the silicon atoms and the amount of the carbon atoms.

The amount of the hydrogen atoms to be incorporated in the surface layer is preferably 41 to 70 atomic %, more preferably 41 to 65 atomic %, and, most preferably, 45 to 60 atomic % respectively to the sum of the

amount of all the constituent atoms to be incorporated in the surface layer.

As long as the amount of the hydrogen atoms to be incorporated in the surface layer lies in the above-mentioned range, any of the resulting light receiving members for use in electrophotography becomes wealthy in significantly practically applicable characteristics and to excel the conventional light receiving members for use in electrophotography in every viewpoint.

That is, for the conventional light receiving member for use in electrophotography, that is known that when there exist certain defects within the surface layer composed of  $A\text{-}(Si_xC_{1-x})_y\text{:H}_{1-y}$  (due to mainly dangling bonds of silicon atoms and those of carbon atoms) they give undesirable influences to the electrophotographic characteristics.

For instance, because of such defects there are often invited deterioration in the electrification characteristics due to charge injection from the side of the free surface, changes in the electrification characteristics due to alterations in the surface structure under certain use environment, for example, high moisture atmosphere, and appearance of residual images upon repeating use due to that an electric charge is injected into the surface layer from the photoconductive layer at the time of corona discharge or at the time of light irradiation to thereby make the electric charge trapped for the defects within the surface layer.

However, the above defects being present in the surface layer of the conventional light receiving member for use in electrophotography which invite various problems as mentioned above can be largely eliminated by controlling the amount of the hydrogen atoms to be incorporated in the surface layer to be more than 41 atomic %, and as a result, the foregoing problems can be almost resolved. In addition, the resulting light receiving member for use in electrophotography becomes to have extremely improved advantages especially in the electric characteristics and the repeating usability at high speed in comparison with the conventional light receiving member for use in electrophotography.

And, the maximum amount of the hydrogen atoms to be incorporated in the surface layer is necessary to be 70 atomic %. That is, when the amount of the hydrogen atoms exceeds 70 atomic %, the hardness of the surface layer is undesirably decreased so that the resulting light receiving member becomes such that can not be repeatedly used for along period of time.

In this connection, it is an essential factor for the light receiving member for use in electrophotography of this invention that the surface layer contains the amount of the hydrogen atoms ranging in the above-mentioned range.

For the incorporation of the hydrogen atoms in said particular amount in the surface layer, it can be carried out by appropriately controlling the related condition such as the flow rate of a starting gaseous substance, the temperature of a substrate, discharging power and the gas pressure.

Specifically, in the case where the surface layer is formed of  $A\text{-}(Si_xC_{1-x})_y\text{:H}_{1-y}$ , the "x" is preferably 0.1 to 0.99999, more preferably 0.1 to 0.99, and, most preferably, 0.15 to 0.9. And the "y" is preferably 0.3 to 0.59, more preferably 0.35 to 0.59, and, most preferably, 0.4 to 0.55.

The thickness of the surface layer in the light receiving member according to this invention is appropriately determined depending upon the desired purpose.

It is, however, also necessary that the layer thickness be determined in view of relative and organic relationships in accordance with the amounts of the halogen atoms, hydrogen atoms and other kind atoms contained in the layer or the characteristics required in the relationship with the thickness of other layer. Further, it should be determined also in economical point of view such as productivity or mass productivity. In view of the above factors, the thickness of the surface layer is preferably 0.003 to 30  $\mu m$ , more preferably, 0.004 to 20  $\mu m$ , and, most preferably, 0.005 to 10  $\mu m$ .

By the way, the thickness of the light receiving layer 100 constituted by the photoconductive layer 103 (or 2103 in FIG. 21) and the surface layer 104 (or 2104 in FIG. 21) in the light receiving member for use in electrophotography according to this invention is appropriately determined depending upon the desired purpose.

In any case, said thickness is appropriately determined in view of relative and organic relationships 20 between the thickness of the photoconductive layer and that of the surface layer so that the various desired characteristics for each of the photoconductive layer and the surface layer in the light receiving member for use in electrophotography can be sufficiently brought about upon the use to effectively attain the foregoing objects of this invention.

And, it is preferred that the thicknesses of the photoconductive layer and the surface layer be determined so that the ratio of the former versus the latter lies in the range of some hundred times to some thousand times.

Specifically, the thickness of the light receiving layer 100 is preferably 3 to 100  $\mu m$ , more preferably 5 to 70  $\mu m$ , and, most preferably, 5 to 50  $\mu m$ .

#### Preparation of Layers

The method of forming the light receiving layer 100 of the light receiving member will be now explained.

Each of the layers to constitute the light receiving layer of the light receiving member of this invention is properly prepared by vacuum deposition method utilizing the discharge phenomena such as glow discharging, sputtering and ion plating methods wherein relevant gaseous starting materials are selectively used.

These production methods are properly used selectively depending on the factors such as the manufacturing conditions, the installation cost required, production scale and properties required for the light receiving members to be prepared. The glow discharging method or sputtering method is suitable since the control for the condition upon preparing the light receiving members having desired properties are relatively easy, and hydrogen atoms, halogen atoms and other atoms can be introduced easily together with silicon atoms. The glow discharging method and the sputtering method may be used together in one identical system.

#### Preparation of Contact Layer, IR Layer, Charge Injection Inhibition Layer, and Photoconductive Layer

Basically, when the charge injection inhibition layer constituted with poly-Si(H,X) or/and the photoconductive layer constituted with A-Si(H,X) are formed, for example, by the glow discharging process, gaseous starting material capable of supplying silico atoms (Si) are introduced together with gaseous starting material 60 for introducing hydrogen atoms (H) and/or halogen atoms (X) into a deposition chamber the inside pressure of which can be reduced, glow discharge is generated in the deposition chamber, and a layer composed of A-

Si(H,X) or/and poly-Si(H,X) are formed on the surface of a substrate placed in a deposition chamber.

In the case of forming such layers by the reactive sputtering process, they are formed by using a Si target and by introducing a gas or gases material capable of supplying halogen atoms (X) or/and hydrogen atoms (H), if necessary, together with an inert gas such as He or Ar into a sputtering deposition chamber to thereby form a plasma atmosphere and then sputtering the Si target.

In the case of forming the IR layer constituted with A-SiGe(H,X) or poly-SiGe(H,X) by the glow discharging process, gaseous starting material capable of supplying silicon atoms (Si) is introduced together with gaseous starting material capable of supplying germanium atoms (Ge), and if necessary gaseous starting material for introducing hydrogen atoms (H) and/or halogen atoms (X) into a deposition chamber the inside pressure of which can be reduced, glow discharge is generated in the deposition chamber, and a layer composed of A-SiGe(H,X) or poly-Si(H,X) is formed on the surface of the substrate placed in the deposition chamber.

To form the IR layer of A-SiGe(H,X) or poly-SiGe(H,X) by the reactive sputtering process, a single target composed of silicon, or two targets (the said target and a target composed of germanium), further a single target composed of silicon and germanium is subjected to sputtering in atmosphere of an inert gas such as He or Ar, and if necessary gaseous starting material capable of supplying germanium atoms diluted with an inert gas such as He or Ar and/or gaseous starting material for introducing hydrogen atoms (H) and/or halogen atoms (X) are introduced into the sputtering deposition chamber thereby forming a plasma atmosphere with the gas.

The gaseous starting material for supplying Si can include gaseous or gasifiable silicon hydrides (silanes) such as SiH<sub>4</sub>, Si<sub>2</sub>H<sub>6</sub>, Si<sub>3</sub>H<sub>8</sub>, Si<sub>4</sub>H<sub>10</sub>, etc., SiH<sub>4</sub> and Si<sub>2</sub>H<sub>6</sub> being particularly preferred in view of the easy layer forming work and the good efficiency for the supply of Si.

The gaseous starting material for supplying Ge can include gaseous or gasifiable germanium hydrides such as GeH<sub>4</sub>, Ge<sub>2</sub>H<sub>6</sub>, Ge<sub>3</sub>H<sub>8</sub>, Ge<sub>4</sub>H<sub>10</sub>, Ge<sub>5</sub>H<sub>12</sub>, Ge<sub>6</sub>H<sub>14</sub>, Ge<sub>7</sub>H<sub>16</sub>, Ge<sub>8</sub>H<sub>18</sub>, and Ge<sub>9</sub>H<sub>20</sub>, etc., GeH<sub>4</sub>, Ge<sub>2</sub>H<sub>6</sub>, and Ge<sub>3</sub>H<sub>8</sub> being particularly preferred in view of the easy layer forming work and the good efficiency for the supply of Ge.

Further, various halogen compounds can be mentioned as the gaseous starting material for introducing the halogen atoms and gaseous or gasifiable halogen compounds, for example, gaseous halogen, halides, inter-halogen compounds and halogen-substituted silane derivatives are preferred. Specifically, they can include halogen gas such as of fluorine, chlorine, bromine, and iodine; inter-halogen compounds such as BrF, ClF, ClF<sub>3</sub>, BrF<sub>2</sub>, BrF<sub>3</sub>, IF<sub>7</sub>, ICl, IBr, etc.; and silicon halides such as SiF<sub>4</sub>, Si<sub>2</sub>F<sub>6</sub>, SiCl<sub>4</sub>, and SiBr<sub>4</sub>.

The use of the gaseous or gasifiable silicon halides as described above for forming a light receiving layer composed of poly-Si or A-Si containing halogen atoms as the constituent atoms by the glow discharging process is particularly advantageous since such layer can be formed with no additional use of gaseous starting material for supplying Si such as silicon hydride.

And, basically, in the case of forming a light receiving layer containing halogen atoms by the glow discharging process, for example, a mixture of a gaseous

silicon halide substance as the starting material for supplying Si and a gas such as Ar, H<sub>2</sub> and He is introduced into the deposition chamber having a substrate in a predetermined mixing ratio and at a predetermined gas flow rate, and the thus introduced gases are exposed to the action of glow discharge to thereby cause a plasma resulting in forming said layer on the substrate. And, for incorporating hydrogen atoms in said layer, an appropriate gaseous starting material for supplying hydrogen atoms can be additionally used.

In the case of forming the IR layer, the above-mentioned halides or halogen-containing silicon compounds can be used as the effective gaseous starting material for supplying halogen atoms. Other examples of the starting material for supplying halogen atoms can include germanium hydride halides such as GeHF<sub>3</sub>, GeH<sub>2</sub>F<sub>2</sub>, GeH<sub>3</sub>F, GeHCl<sub>3</sub>, GeH<sub>2</sub>Cl<sub>2</sub>, GeH<sub>3</sub>Cl, GeHBr<sub>3</sub>, GeH<sub>2</sub>Br<sub>2</sub>, GeH<sub>3</sub>Br, GeHI<sub>3</sub>, GeH<sub>2</sub>I<sub>2</sub>, and GeH<sub>3</sub>I; and germanium halides such as GeF<sub>4</sub>, GeCl<sub>4</sub>, GeBr<sub>4</sub>, GeI<sub>4</sub>, GeF<sub>2</sub>, GeCl<sub>2</sub>, GeBr<sub>2</sub>, and GeI<sub>2</sub>. They are in the gaseous form or gasifiable substances.

And in any case, one of these gaseous or gasifiable starting materials or a mixture of two or more of them in a predetermined mixing ratio can be selectively used.

As above mentioned, in the case of forming a layer composed constituted with, for example, poly-Si(H,X) or A-Si(H,X) by the reactive sputtering process, such layer is formed on the substrate by using an Si target and sputtering the Si target in a plasma atmosphere.

And, in order to form such layer by the ion-plating process, the vapor of polycrystal silicon or single crystal silicon is allowed to pass through a desired gas plasma atmosphere. The silicon vapor is produced by heating the polycrystal silicon or single crystal silicon held in a boat. The heating is accomplished by resistance heating or in accordance with the electron beam method (E.B. method).

In either case where the sputtering process or the ion-plating process is employed, the layer may be incorporated with halogen atoms by introducing one of the above-mentioned gaseous halides or halogen-containing silicon compounds into the deposition chamber in which a plasma atmosphere of the gas is produced. In the case where the layer is incorporated with hydrogen atoms in accordance with the sputtering process, a feed gas to liberate hydrogen is introduced into the deposition chamber in which a plasma atmosphere of the gas is produced. The feed gas to liberate hydrogen atoms includes H<sub>2</sub> gas and the above-mentioned silanes.

As for the gaseous or gasifiable starting material for incorporating halogen atoms in the IR layer, charge injection inhibition layer or photoconductive layer, the foregoing halide, halogen-containing silicon compound or halogen-containing germanium compound can be effectively used. Other effective examples of said material can include hydrogen halides such as HF, HCl, HBr and HI and halogen-substituted silanes such as SiH<sub>2</sub>F<sub>2</sub>, SiH<sub>2</sub>I<sub>2</sub>, SiH<sub>2</sub>Cl<sub>2</sub>, SiHCl<sub>3</sub>, SiH<sub>2</sub>Br<sub>2</sub> and SiHBr<sub>3</sub>, which contain hydrogen atom as the constituent element and which are in the gaseous state or gasifiable substances. The use of the gaseous or gasifiable hydrogen-containing halides is particularly advantageous since, at the time of forming a light receiving layer, the hydrogen atoms, which are extremely effective in view of controlling the electrical or photoelectrographic properties, can be introduced into that layer together with halogen atoms.

The structural introduction of hydrogen atoms into the layer can be carried out by introducing, in addition to these gaseous starting materials, H<sub>2</sub>, or silicon hydrides such as SiH<sub>4</sub>, SiH<sub>6</sub>, Si<sub>3</sub>H<sub>6</sub>, Si<sub>4</sub>H<sub>10</sub>, etc. into the deposition chamber together with a gaseous or gasifiable silicon-containing substance for supplying Si, and producing a plasma atmosphere with these gases therein.

The amount of the hydrogen atoms (H) and/or the amount of the halogen atoms (X) to be contained in the layer are adjusted properly by controlling related conditions, for example, the temperature of a substrate, the amount of a gaseous starting material capable of supplying the hydrogen atoms or the halogen atoms into the deposition chamber and the electric discharging power.

In order to incorporate the group III atoms or the group V atoms, and, oxygen atoms, nitrogen atoms or carbon atoms in the IR layer, the charge injection inhibition layer or the photoconductive layer using the glow discharging process, reactive sputtering process or ion plating process, the starting material capable of supplying the group III or group V atoms, and, the starting material capable of supplying oxygen atoms, nitrogen atoms or carbon atoms are selectively used together with the starting material for forming the IR layer, the charge injection inhibition layer or the photoconductive layer upon forming such layer while controlling the amount of them in that layer to be formed.

As the starting material to introduce the atoms (O, N, C), many gaseous or gasifiable substances containing any of oxygen, carbon, and nitrogen atoms as the constituent atoms can be used. Likewise, as for the starting material to introduce the group III or group V atoms, many gaseous or gasifiable substances can be used.

For example, referring to the starting material for introducing oxygen atoms, most of those gaseous or gasifiable materials which contain at least oxygen atoms as the constituent atoms can be used.

And, it is possible to use a mixture of a gaseous starting material containing silicon atoms (Si) as the constituent atoms, a gaseous starting material containing oxygen atoms (O) as the constituent atom and, as required, a gaseous starting material containing hydrogen atoms (H) and/or halogen atoms (X) as the constituent atoms in a desired mixing ratio, a mixture of gaseous starting material containing silicon atoms (Si) as the constituent atoms and a gaseous starting material containing oxygen atoms (O) and hydrogen atoms (H) as the constituent atoms in a desired mixing ratio, or a mixture of gaseous starting material containing silicon atoms (Si) as the constituent atoms and a gaseous starting material containing silicon atoms (Si), oxygen atoms (O) and hydrogen atoms (H) as the constituent atoms.

Further, it is also possible to use a mixture of a gaseous starting material containing silicon atoms (Si) and hydrogen atoms (H) as the constituent atoms and a gaseous starting material containing oxygen atoms (O) as the constituent atoms.

Specifically, there can be mentioned, for example, oxygen (O<sub>2</sub>), ozone (O<sub>3</sub>), nitrogen monoxide (NO), nitrogen dioxide (NO<sub>2</sub>), dinitrogen oxide (N<sub>2</sub>O), dinitrogen trioxide (N<sub>2</sub>O<sub>3</sub>), dinitrogen tetraoxide (N<sub>2</sub>O<sub>4</sub>), dinitrogen pentoxide (N<sub>2</sub>O<sub>5</sub>), nitrogen trioxide (NO<sub>3</sub>), lower siloxanes comprising silicon atoms (Si), oxygen atoms (O) and hydrogen atoms (H) as the constituent atoms, for example, disiloxane (H<sub>3</sub>SiOSiH<sub>3</sub>) and trisiloxane (H<sub>3</sub>SiOSiH<sub>2</sub>OSiH<sub>3</sub>), etc.

Likewise, as the starting material for introducing nitrogen atoms, most of gaseous or gasifiable materials which contain at least nitrogen atoms as the constituent atoms can be used.

For instance, it is possible to use a mixture of a gaseous starting material containing silicon atoms (Si) as the constituent atoms, a gaseous starting material containing nitrogen atoms (N) as the constituent atoms and, optionally, a gaseous starting material containing hydrogen atoms (H) and/or halogen atoms (X) as the constituent atoms in a desired mixing ratio, or a mixture of a starting gaseous material containing silicon atoms (Si) as the constituent atoms and a gaseous starting material containing nitrogen atoms (N) and hydrogen atoms (H) as the constituent atoms also in a desired mixing ratio.

Alternatively, it is also possible to use a mixture of a gaseous starting material containing nitrogen atoms (N) as the constituent atoms and a gaseous starting material containing silicon atoms (Si) and hydrogen atoms (H) as the constituent atoms.

The starting material that can be used effectively as the gaseous starting material for introducing the nitrogen atoms (N) used upon forming the layer containing nitrogen atoms can include gaseous or gasifiable nitrogen, nitrides and nitrogen compounds such as azide compounds comprising N as the constituent atoms or N and H as the constituent atoms, for example, nitrogen (N<sub>2</sub>), ammonia (NH<sub>3</sub>), hydrazine (H<sub>2</sub>NNH<sub>2</sub>) hydrogen azide (HN<sub>3</sub>) and ammonium azide (NH<sub>4</sub>N<sub>3</sub>). In addition, nitrogen halide compounds such as nitrogen trifluoride (F<sub>3</sub>N) and nitrogen tetrafluoride (F<sub>4</sub>N<sub>2</sub>) can also be mentioned in that they can also introduce halogen atoms (X) in addition to the introduction of nitrogen atoms (N).

Further, as for the starting material for introducing carbon atoms, gaseous or gasifiable materials containing carbon atoms as the constituent atoms can be used.

And it is possible to use a mixture of gaseous starting material containing silicon atoms (Si) as the constituent atoms, gaseous starting material containing carbon atoms (C) as the constituent atoms and, optionally, gaseous starting material containing hydrogen atoms (H) and/or halogen atoms (X) as the constituent atoms in a desired mixing ratio, a mixture of gaseous starting material containing silicon atoms (Si) as the constituent atoms and gaseous starting material containing carbon atoms (C) and hydrogen atoms (H) as the constituent atoms also in a desired mixing ratio, or a mixture of gaseous starting material containing silicon atoms (Si) as the constituent atoms and gaseous starting material comprising silicon atoms (Si).

Those gaseous starting materials that are effectively usable herein can include gaseous silicon hydrides containing carbon atoms (C) and hydrogen atoms (H) as the constituent atoms, such as silanes, for example, SiH<sub>4</sub>, Si<sub>2</sub>H<sub>6</sub>, Si<sub>3</sub>H<sub>8</sub> and Si<sub>4</sub>H<sub>10</sub>, as well as those containing carbon atoms (C) and hydrogen atoms (H) as the constituent atoms, for example, saturated hydrocarbons of 1 to 4 carbon atoms, ethylenic hydrocarbons of 3 to 4 carbon atoms and acetylenic hydrocarbons of 2 to 3 carbon atoms.

Specifically, the saturated hydrocarbons can include methane (CH<sub>4</sub>), ethane (C<sub>2</sub>H<sub>6</sub>), propane (C<sub>3</sub>H<sub>8</sub>), n-butane (n-C<sub>4</sub>H<sub>10</sub>) and pentane (C<sub>5</sub>H<sub>12</sub>), the ethylenic hydrocarbons can include ethylene (C<sub>2</sub>H<sub>4</sub>), propylene (C<sub>3</sub>H<sub>6</sub>), butene-1 (C<sub>4</sub>H<sub>8</sub>), butene-2 (C<sub>4</sub>H<sub>8</sub>), isobutylene (C<sub>4</sub>H<sub>8</sub>) and pentene (C<sub>5</sub>H<sub>10</sub>) and the acetylenic hydro-

carbons can include acetylene ( $C_2H_2$ ), methylacetylene ( $C_3H_4$ ) and butine ( $C_4H_6$ ).

The gaseous starting material containing silicon atoms (Si), carbon atoms (C) and hydrogen atoms (H) as the constituent atoms can include silicided alkyls, for example,  $Si(CH_3)_4$  and  $Si(C_2H_5)_4$ . In addition to these gaseous starting materials,  $H_2$  can of course be used as the gaseous starting material for introducing hydrogen atoms (H).

In order to form the IR layer, the charge injection prohibition layer or the photoconductive layer incorporated with the group III or group V atoms using the glow discharging process, reactive sputtering process or ion plating process, the starting material for introducing the group III or group V atoms is used together with the starting material for forming such upon forming that layer while controlling the amount of them in the layer to be formed.

For instance, in the case of forming a layer composed of poly- $Si(H,X)$  or of A- $Si(H,X)$  containing the group III or group V atoms, namely poly- $SiM(H,X)$  or A- $SiM(H,X)$  wherein M stands for the group III or group V atoms, by using the glow discharging, the starting gases material for forming such layer are introduced into a deposition chamber in which a substrate being placed, optionally being mixed with an inert gas such as Ar or He in a predetermined mixing ratio, and the thus introduced gases are exposed to the action of glow discharge to thereby cause a gas plasma resulting in forming a layer composed of a- $SiM(H,X)$  on the substrate.

Referring specifically to the boron atom introducing materials as the starting material for introducing the group III atoms, they can include boron hydrides such as  $B_2H_6$ ,  $B_4H_{10}$ ,  $B_5H_9$ ,  $B_5H_{11}$ ,  $B_6H_{10}$ ,  $B_6H_{12}$  and  $B_6H_{14}$  and boron halides such as  $BF_3$ ,  $BCl_3$  and  $BBr_3$ . In addition,  $AlCl_3$ ,  $CaCl_3$ ,  $Ga(CH_3)_2$ ,  $InCl_3$ ,  $TiCl_3$  and the like can also be mentioned.

Referring to the starting material for introducing the group V atoms and, specifically, to the phosphorus atom introducing materials, they can include, for example, phosphor hydrides such as  $PH_3$  and  $P_2H_6$  and phosphor halide such as  $PH_4I$ ,  $PF_3$ ,  $PF_5$ ,  $PCl_3$ ,  $PCl_5$ ,  $PBr_3$ ,  $PBr_5$  and  $PI_3$ . In addition,  $AsH_3$ ,  $AsF_5$ ,  $AsCl_3$ ,  $AsBr_3$ ,  $AsF_3$ ,  $SbH_3$ ,  $SbF_3$ ,  $SbF_5$ ,  $SbCl_3$ ,  $SbCl_5$ ,  $BiH_3$ ,  $SiCl_3$  and  $BiBr_3$  can also be mentioned to as the effective starting material for introducing the group V atoms.

The amount of the group III or group V atoms to be contained in the IR layer, the charge injection prohibition layer or the photoconductive layer are adjusted properly by controlling the related conditions, for example, the temperature of a substrate, the amount of a gaseous starting material capable of supplying the group III or group V atoms, the gas flow rate of such gaseous starting material, the discharging power, the inner pressure of the deposition chamber, etc.

The conditions upon forming the constituent layers of the light receiving member of the invention, for example, the temperature of the support, the gas pressure in the deposition chamber, and the electric discharging power are important factors for obtaining the light receiving member having desired properties and they are properly selected while considering the function of each of the layers to be formed. Further, since these layer forming conditions may be varied depending on the kind and the amount of each of the atoms contained in the layer, the conditions have to be determined also

taking the kind or the amount of the atoms to be contained into consideration.

Specifically, the conditions upon forming the constituent layer of the light receiving member of this invention are different according to the kind of the material with which the layer is to be constituted.

In the case of forming the charge injection inhibition layer which is constituted with a poly-Si material, and the IR layer which is constituted also with a poly-Si material in case where necessary, the relationship between the temperature of a substrate and the electrical discharging power is extremely important.

That is, when the temperature of the substrate is adjusted to be in the range from 200° to 350° C., the electrical discharging power is adjusted to be preferably in the range from 1100 to 5000 W/cm<sup>2</sup>, and more preferably, in the range 1500 to 4000 W/cm<sup>2</sup>. And, when the temperature of the substrate is adjusted to be in the range from 350° to 700° C., the electrical discharging power is adjusted to be preferably in the range from 100 to 5000 W/cm<sup>2</sup>, and more preferably in the range from 200 to 4000 W/cm<sup>2</sup>.

And as for the gas pressure in the deposition chamber in the above case, it is preferably  $10^{-3}$  to  $8 \times 10^{-1}$  Torr, and more preferably,  $5 \times 10^{-3}$  to  $5 \times 10^{-1}$  Torr.

On the other hand, in the case of forming the photoconductive layer which is constituted with an A-Si material, and the IR layer which is constituted also with an A-Si material, the temperature of the substrate is usually from 50° to 350° C., preferably, from 50° to 300° C., most suitably 100° to 250° C.; the gas pressure in the deposition chamber is usually from  $1 \times 10^{-2}$  to 5 Torr, preferably, from  $1 \times 10^{-2}$  to 3 Torr, most suitably from  $1 \times 10^{-2}$  to 1 Torr; and the electrical discharging power is preferably from 10 to 1000 W/cm<sup>2</sup>, and more preferably, from 20 to 500 W/cm<sup>2</sup>.

In any case, the actual conditions for forming the layer such as temperature of the support, discharging power and the gas pressure in the deposition chamber cannot usually be determined with ease independent of each other. Accordingly, the conditions optimal to the layer formation are desirably determined based on relative and organic relationships for forming the corresponding layer having desired properties.

#### Preparation of Surface Layer

The surface layer 104 in the light receiving member for use in electrophotography according to this invention is constituted with an amorphous material composed of A-( $Si_xC_{1-x})_y$ ;  $H_{1-y}$  [ $x > 0$ ,  $y < 1$ ] which contains 41 to 70 atomic % of hydrogen atoms and is disposed on the above-mentioned photoconductive layer.

The surface layer can be properly prepared by vacuum deposition method utilizing the discharge phenomena such as flow discharging, sputtering or ion plating wherein relevant gaseous starting materials are selectively used as well as in the above-mentioned cases for preparing the photoconductive layer.

However, the glow discharging method or sputtering method is suitable since the control for the condition upon preparing the surface layer having desired properties are relatively easy, and hydrogen atoms and carbon atoms can be introduced easily together with silicon atoms. The glow discharging method and the sputtering method may be used together in an identical system.

Basically, when a layer constituted with A-( $Si_xC_{1-x})_y$ ;  $H_{1-y}$  is formed, for example, by the glow discharging method, gaseous starting material capable

of supplying silicon atoms (Si) are introduced together with a gaseous starting material for introducing hydrogen atoms (H) and/or halogen atoms (X) into a deposition chamber the inside pressure of which can be reduced, glow discharge is generated in the deposition chamber, and a layer constituted with A-(Si<sub>x</sub>C<sub>1-x</sub>)<sub>y</sub>:H<sub>1-y</sub> containing 41 to 70 atomic % of hydrogen atoms is formed on the surface of a substrate placed in the deposition chamber.

As for the gaseous starting materials for supplying silicon atoms (Si) and/or hydrogen atoms (H), the same gaseous materials as mentioned in the above cases for preparing photoconductive layer can be used as long as they do not contain any of halogen atoms, nitrogen atoms and oxygen atoms.

That is, the gaseous starting material usable for forming the surface layer can include almost any kind of gaseous or gasifiable materials as far as it contains one or more kinds selected from silicon atoms, hydrogen atoms and carbon atoms as the constituent atoms.

Specifically, for the preparation of the surface layer, it is possible to use a mixture of gaseous starting material containing silicon atoms (Si) as the constituent atoms, gaseous starting material containing carbon atoms (C) as the constituent atoms and, optionally, gaseous starting material containing hydrogen atoms (H) as the constituent atoms in a desired mixing ratio, a mixture of gaseous starting material containing silicon atoms (Si) as the constituent atoms and gaseous starting material containing carbon atoms (C) and hydrogen atoms (H) as the constituent atoms also in a desired mixing ratio, or a mixture of gaseous starting material containing silicon atoms (Si) as the constituent atoms and gaseous starting material comprising silicon atoms (Si) in the glow discharging process as described above.

Those gaseous starting materials that are effectively usable herein can include gaseous silicon hydrides containing carbon atoms (C) and hydrogen atoms (H) as the constituent atoms, such as silanes, for example, SiH<sub>4</sub>, Si<sub>2</sub>H<sub>6</sub>, Si<sub>3</sub>H<sub>8</sub> and Si<sub>4</sub>H<sub>10</sub>, as well as those containing carbon atoms (C) and hydrogen atoms (H) as the constituent atoms, for example, saturated hydrocarbons of 1 to 4 carbon atoms, ethylenic hydrocarbons of 2 to 4 carbon atoms and acetylenic hydrocarbons of 2 to 3 carbon atoms.

Specifically, the saturated hydrocarbons can include methane (CH<sub>4</sub>), ethane (C<sub>2</sub>H<sub>6</sub>), propane (C<sub>3</sub>H<sub>8</sub>), n-butane (n-C<sub>4</sub>H<sub>10</sub>) and pentane (C<sub>5</sub>H<sub>12</sub>), the ethylenic hydrocarbons can include ethylene (C<sub>2</sub>H<sub>4</sub>), propylene (C<sub>3</sub>H<sub>6</sub>), butene-1 (C<sub>4</sub>H<sub>8</sub>), butene-2 (C<sub>4</sub>H<sub>8</sub>), isobutylene (C<sub>4</sub>H<sub>8</sub>) and pentene (C<sub>5</sub>H<sub>10</sub>) and the acetylenic hydrocarbons can include acetylene (C<sub>2</sub>H<sub>2</sub>), methylacetylene (C<sub>3</sub>H<sub>4</sub>) and butine (C<sub>4</sub>H<sub>6</sub>).

The gaseous starting material containing silicon atoms (Si), carbon atoms (C) and hydrogen atoms (H) as the constituent atoms can include silicided alkyls, for example, Si(CH<sub>3</sub>)<sub>4</sub> and Si(C<sub>2</sub>H<sub>5</sub>)<sub>4</sub>. In addition to these gaseous starting materials, H<sub>2</sub> can of course be used as the gaseous starting material for introducing hydrogen atoms (H).

In the case of forming the surface layer by way of the sputtering process, it is carried out by using a single crystal or polycrystalline Si wafer, a C (graphite) wafer or a wafer containing a mixture of Si and C as a target and sputtering them in a desired gas atmosphere.

In the case of using, for example, an Si wafer as a target, a gaseous starting material for introducing carbon atoms (C) is introduced while being optionally diluted with a dilution gas such as Ar and He into a

sputtering deposition chamber thereby forming gas plasmas with these gases and sputtering the Si wafer.

Alternatively, in the case of using Si and C as individual targets or as a single target comprising Si and C in admixture, gaseous starting material for introducing hydrogen atoms as the sputtering gas is optionally diluted with a dilution gas, introduced into a sputtering deposition chamber thereby forming gas plasmas and sputtering is carried out. As the gaseous starting material for introducing each of the atoms used in the sputtering process, those gaseous starting materials used in the glow discharging process as described above may be used as they are.

The conditions upon forming the surface layer constituted with an amorphous material composed of A-(Si<sub>x</sub>C<sub>1-x</sub>)<sub>y</sub>:H<sub>1-y</sub> which contains 41 to 71 atomic % of hydrogen atoms, for example, the temperature of the substrate, the gas pressure in the deposition chamber and the electric discharging power are important factors for obtaining a desirable surface layer having desired properties and they are properly selected while considering the functions of the layer to be formed. Further, since these layer forming conditions may be varied depending on the kind and the amount of each of the atoms contained in the light receiving layer, the conditions have to be determined also taking the kind or the amount of the atoms to be contained into consideration.

Specifically, the temperature of the substrate is preferably from 50° to 350° C. and, most preferably, from 100° to 300° C. The gas pressure in the deposition chamber is preferably from 0.01 to 1 Torr and, most preferably, from 0.1 to 0.5 Torr. Further, the electrical discharging power is preferably from 10 to 1000 W/cm<sup>2</sup>, and, most preferably, from 20 to 500 W/cm<sup>2</sup>.

However, the actual conditions for forming the surface layer such as the temperature of a substrate, discharging power and the gas pressure in the deposition chamber can not usually be determined with ease independent of each other. Accordingly, the conditions optimal to the formation of the surface layer are desirably determined based on relative and organic relationships for forming the surface layer having desired properties.

#### 45 DESCRIPTION OF THE PREFERRED EMBODIMENTS

The invention will be described more specifically while referring to Examples 1 through 24, but the invention is not intended to limit the scope only to these examples.

In each of the examples, the light receiving layer was formed by using the glow discharging process. FIG. 24 shows the apparatus for preparing the light receiving member according to this invention.

Gas reservoirs 2402, 2403, 2404, 2405, and 2406 illustrated in the figure are charged with gaseous starting materials for forming the respective layers in the light receiving member for use in electrophotography according to this invention, that is, for instance, SiH<sub>4</sub> gas (99.99% purity) in the reservoir 2402, B<sub>2</sub>H<sub>6</sub> gas (99.999% purity) diluted with H<sub>2</sub> (referred to as "B<sub>2</sub>H<sub>6</sub>/H<sub>2</sub>") in the reservoir 2403, H<sub>2</sub> gas (99.99999% purity) in the reservoir 2404, NO gas (99.999% purity) in the reservoir 2405, and CH<sub>4</sub> gas (99.99% purity) in the reservoir 2406.

Prior to the entrance of these gases into a reaction chamber 2401, it is confirmed that valves 2422-2426 for

the gas reservoirs 2402-2406 and a leak valve 2435 are closed and that inlet valves 2412-2416, exit valves 2417-2421, and sub-valves 2432 and 2433 are opened. Then, a main valve 2434 is at first opened to evacuate the inside of the reaction chamber 2401 and gas piping.

Then, upon observing that the reading on the vacuum 2436 became about  $5 \times 10^{-6}$  Torr, the sub-valves 2432 and 2433 and the exit valves 2417 through 2421 are closed.

Now, reference is made to the example shown in FIG. 1(A) in the case of forming the photo receiving layer on an Al cylinder as a substrate 3437.

At first, SiH<sub>4</sub> gas from the gas reservoir 2402, B<sub>2</sub>H<sub>6</sub>/H<sub>2</sub> gas from the gas reservoir 2403, H<sub>2</sub> gas from the gas reservoir 2404, and NO gas from the gas reservoir 2505 are caused to flow into mass flow controllers 2407, 2408, 2409, and 2410 respectively by opening the inlet valves 412, 2413, 2414, and 2415, controlling the pressure of exit pressure gauges 2427, 2428, 2429, and 2430 to 1 kg/cm<sup>2</sup>. Subsequently, the exit valves 2417, 2418, 2419, and 2420, and the sub-valve 2432 are gradually opened to enter the gases into the reaction chamber 2401. In this case, the exit valves 2417, 2418, 2419, and 2420 are adjusted so as to attain a desired value for the ratio among the SiH<sub>4</sub> gas flow rate, NO gas flow rate, CH<sub>4</sub> gas flow rate, and B<sub>2</sub>H<sub>6</sub>/H<sub>2</sub> gas flow rate and the opening of the main valve 2434 is adjusted while observing the reading on the vacuum gauge 2436 so as to obtain a desired value for the pressure inside the reaction chamber 2401. Then, after confirming that the temperature of the 2437 has been set by a heater 2448 within a range from 50° to 350° C., a power source 2440 is set to a predetermined electrical power to cause glow discharging in the reaction chamber 2401 while controlling the flow rates of NO gas and/or B<sub>2</sub>H<sub>6</sub>/H<sub>2</sub> gas in accordance with a previously designed variation coefficient curve by using a microcomputer (not shown), thereby forming, at first, a charge injection inhibition layer 102 containing oxygen atoms and boron atoms on the substrate cylinder 2437. When the layer 102 has reached a desired thickness, the exit valves 2418 and 2420 are completely closed to stop B<sub>2</sub>H<sub>6</sub>/H<sub>2</sub> gas and NO gas into the deposition chamber 2401. At the same time, the flow rate of SiH<sub>4</sub> gas and the flow rate of H<sub>2</sub> gas are controlled by regulating the exit valves 2417 and 2419 and the layer formation process is continued to thereby form a photoconductive layer without containing both oxygen atoms and boron atoms having a desired thickness on the previously formed charge injection inhibition layer.

In the case of forming a photoconductive layer containing oxygen atoms and/or boron atoms, the flow rate for the gaseous starting material to supply such atoms in appropriately controlled in stead of closing the exit valves 2418 and/or 2420.

In the case where halogen atoms are incorporated in the charge injection inhibition layer 102 and the photoconductive layer 103, for example, SiF<sub>4</sub> gas is fed into the reaction chamber 2401 in addition to the gases as mentioned above.

And it is possible to further increase the layer forming speed according to the kind of a gas to be selected. For example, in the case wher the charge injection inhibition layer 102 and the photoconductive layer 103 are formed using Si<sub>2</sub>H<sub>6</sub> gas in stead of the SiH<sub>4</sub> gas, the layer forming speed can be increased by a few holds and as a result, the layer productivity can be rised.

In order to form the surface layer 104 or the resulting photoconductive layer, for example, SiH<sub>4</sub> gas, CH<sub>4</sub> gas and if necessary, a dilution gas such as H<sub>2</sub> gas are intro-

duced into the reaction chamber 2401 by operating the corresponding valves in the same manner as in the case of forming the photoconductive layer and glow discharging is caused therein under predetermined conditions to thereby form the surface layer.

In that case, the amount of the carbon atoms to be incorporated in the surface layer can be properly controlled by appropriately changing the flow rate for the SiH<sub>4</sub> gas and that for the CH<sub>4</sub> gas respectively to be introduced into the reaction chamber 2401. As for the amount of the hydrogen atoms to be incorporated in the surface layer, it can be properly controlled by appropriately changing the flow rate of the H<sub>2</sub> gas to be introduced into the reaction chamber 2401.

All of the exit valves other than those required for upon forming the respective layers are of course closed. Further, upon forming the respective layers, the inside of the system is once evacuated to a high vacuum degree as required by closing the exit valves 2417 through 2421 while entirely opening the sub-valve 2432 and entirely opening the main valve 2434.

Further, during the layer forming operation, the Al cylinder as substrate 2437 is rotated at a predetermined speed by the action of the motor 2439.

#### EXAMPLE 1

A light receiving member for use in electrophotography having a light receiving layer disposed on an Al cylinder having a mirror grinded surface was prepared under the layer forming conditions shown in Table 1 using the fabrication apparatus shown in FIG. 24.

And, a sample having only a surface layer on the same kind Al cylinder and another sample having only a charge injection inhibition layer on the same kind Al cylinder respectively as in the above case were prepared respectively in the same manner for forming the surface layer and in the same manner for forming the charge injection prohibition layer in the above case using the same kind fabrication apparatus as shown in FIG. 24.

For the resulting light receiving member (hereinafter, this kind light receiving member is referred to as "drum"), it was set with the conventional electrophotographic copying machine, and electrophotographic characteristic such as initial electrification efficiency, residual voltage and appearance of a ghost were examined, then decrease in the electrification efficiency, deterioration on photosensitivity and increase of defective images after 1,500 thousand times repeated shots were respectively examined.

Further, the situation of an image flow on the drum under high temperature and high humidity atmosphere at 35° C. and 85% humidity was also examined.

As for the resulting sample having only the surface layer, upper part, middle part and lower part of its image forming part were cut off, and were engaged in quantitative analysis by the conventional organic element analyzer to analize the content of hydrogen atoms in each of the cut-off parts.

As for the resulting sample having only the charge injection prohibition layer, in the same way as the above sample, upper part, middle part and lower part were cut off, and were subjected to the measurement of diffraction patterns corresponding to Si (111) near 27° of the diffraction angle by the conventional X-ray diffractometer to examine the existence of crystallinity.

The results of the various evaluations, the results of the quantitative analysis of the content of the hydrogen

atoms, and the situations of crystallinity for the samples are as shown in Table 2.

As Table 2 illustrates, considerable advantages on items of initial electrification efficiency, effective image flow and sensitivity deterioration were acknowledged.

#### COMPARATIVE EXAMPLE 1

Except that the layer forming conditions changed as shown in Table 3, the drum and the sample were made under the same fabrication apparatus and manner as Example 1 and were provided to examine the same items. The results are shown in Table 4. As the Table 4 illustrates, much defects on various items were acknowledged compared to the case of Example 1.

#### EXAMPLE 2

A light receiving member for use in electrophotography having a light receiving layer 100 disposed on an Al cylinder having a mirror grinded surface was prepared under the layer forming conditions shown in Table 5 using the fabrication apparatus shown in FIG. 24.

And a sample having only a surface layer on the same kind Al cylinder as in the above case was prepared in the same manner for forming the surface layer in the above case using the same kind fabrication apparatus as shown in FIG. 24.

Likewise, another sample having only a charge injection prohibition layer was prepared.

For the resulting light receiving member, it was set with the conventional electrophotographic copying machine, and electrophotographic characteristics such as initial electrification efficiency, residual voltage and appearance of a ghost were examined, then decrease in the electrification efficiency, deterioration on photosensitivity and increase of defective images after 1,500 thousand times repeated shots were respectively examined.

Further, the situation of an image flow or the drum under high temperature and high humidity atmosphere at 35° C. and 85% humidity was also examined.

As for the resulting former sample, a middle part was cut off and subjected to the analysis of the component's thicknesswise distribution by IMA.

Then, a middle part was cut off from the drum, and it was subjected to the analysis of the element's thicknesswise distribution by IMA.

As for the resulting former sample, upper part, middle part and lower part of its image forming part were cut off, and were engaged in quantitative analysis by the conventional organic element analyzer to analyze the content of hydrogen atoms in each of the cut-off parts.

As for the latter sample, in the same way as the above case, upper part, middle part and lower part were cut off, and were subjected to the measurement of diffraction patterns corresponding to Si (111) near 27° of the diffraction angle by the conventional X-ray diffractometer to examine the existence of crystallinity.

The results of the various evaluations, the results of the quantitative analysis of the content of the hydrogen atoms and the situation of crystallinity for the samples are shown in Table 6.

And, the elements profiles in the thicknesswise direction of the boron atoms (B) and the oxygen atoms (O) are shown in FIG. 27.

As Table 6 illustrates, considerable advantages on items of initial electrification efficiency, effective image flow and sensitivity deterioration were acknowledged.

#### EXAMPLE 3 (CONTAINING COMPARATIVE EXAMPLE 2)

Multiple drums and samples for analysis were provided under the same conditions as in Example 1, except the conditions for forming a surface layer were changed to those shown in Table 7.

As a result of subjecting these drums and samples to the same evaluations and analyses as in Example 1, the results shown in Table 8 were obtained.

#### EXAMPLE 4

With the layer forming conditions for a photoconductive layer changed to the figures of Table 9, multiple drums having a light receiving layer under the same conditions as in Example 1 were provided. These drums were examined by the same procedures as in Example 1. The results are shown in Table 10.

#### EXAMPLE 5

With the layer forming conditions for a charge injection inhibition layer changed to the figures of Table 11, multiple drums having a light receiving layer and samples having only a charge injection prohibition layer were provided under the same conditions as in Example 1. And they were examined by the same procedures as in Example 1. The results are shown in Table 12.

With the layer forming conditions for a charge injection inhibition layer changed to the figures of Table 13, multiple drums having a light receiving layer and samples having only a charge injection prohibition layer were provided under the same conditions as in Example 1. And they were examined by the same procedures as in Example 1. The results are shown in Table 14.

#### EXAMPLE 7

There were prepared multiple light receiving members respectively having a contact layer formed under the different layer forming conditions as shown in Table 15 and a light receiving layer formed under the same layer forming conditions as in Example 1 respectively on the same kind Al cylinder as in Example 1.

And samples having only a contact layer were prepared in the same procedures as in the above case.

As for the resulting light receiving members, there were evaluated by the same procedures as in Example 1. As for the resulting samples, they were subjected to the measurement of diffraction patterns corresponding to Si (111) near 27° of the diffraction angle by the conventional X-ray diffractometer to examine the existence of crystallinity.

The results are shown in Table 16.

#### EXAMPLE 8

There were prepared multiple light receiving members respectively having a contact layer formed under the different layer forming conditions as shown in Table 17 and a light receiving layer formed under the same layer forming conditions as in Example 1 respectively on the same kind Al cylinder as in Example 1.

They were evaluated by the same procedures as in Example 1.

The results are shown in Table 18.

#### EXAMPLE 9

The mirror grinded cylinders were supplied for grinding process of cutting tool of various degrees. With the patterns of FIG. 25, various cross section

patterns as described in Table 19 multiple cylinders were provided. These cylinders were set to the fabrication apparatus of FIG. 24 accordingly, and used to produce drums under the same layer forming conditions of Example 1. The resulting drums were evaluated with the conventional electrophotographic copying machine having digital exposure functions and using semiconductor laser of 780 nm wavelength. The results are shown in Table 20.

#### EXAMPLE 10

The surface of mirror grinded cylinder was treated by dropping lots of bearing balls thereto to thereby form uneven shape composed of a plurality of fine dimples at the surface, and multiple cylinders having a cross section form of FIG. 26 and of a cross section pattern of Table 21 were provided. These cylinders were set to the fabrication apparatus of FIG. 24 accordingly and used for the preparation of drums under the same layer forming conditions of Example 1. The resulting drums are evaluated with the conventional electrophotographic copying machine having digital exposure functions and using semiconductor laser of 780 nm wavelength. The results are shown in Table 22.

#### EXAMPLE 11

A light receiving member for use in electrophotography having a light receiving layer disposed on an Al cylinder having a mirror grinded surface was prepared under the layer forming conditions shown in Table 33 using the fabrication apparatus shown in FIG. 24.

And, a sample having only a surface layer on the same kind Al cylinder, another sample having only a charge injection inhibition layer on the same kind Al cylinder and further sample having only an IR layer on the same kind Al cylinder respectively as in the above case were prepared respectively in the same manners for forming the surface for forming the charge injection inhibition layer and for forming the IR layer in the above case using the same kind fabrication apparatus as shown in FIG. 24.

For the resulting light receiving member, it was set with the conventional electrophotographic copying machine, and electrophotographic characteristics such as initial electrification efficiency, residual voltage and appearance of a ghost were examined, then decrease in the electrification efficiency, deterioration on photosensitivity and increase of defective images after 1,500 thousand times repeated shots were respectively examined.

Further, the situation of an image flow on the drum under high temperature and high humidity atmosphere at 35° C. and 85% humidity was also examined.

As for the resulting first sample having only the surface layer, upper part, idle part and lower part of its image forming part were cut off, and were engaged in quantitative analysis by the conventional organic element analyzer to analize the content of hydrogen atoms in each of the cut-off parts.

As for the resulting second sample having only the charge injection prohibition layer and the resulting third sample having only the IR layer, in the same way as the above sample, upper part, middle part and lower part were cut off for each sample, and were subjected to the measurement of diffraction patterns corresponding to Si (111) near 27° of the diffraction angle by the conventional X-ray diffractometer to examine the existence of crystallinity.

The results of the various evaluation, the results of the quantitative analysis of the content of the hydrogen atoms, and the situations of crystallinity for the samples are as shown in Table 24.

As Table 24 illustrates, considerable advantages on items of initial electrification efficiency, effective image flow and sensitivity deterioration were acknowledged.

#### COMPARATIVE EXAMPLE 3

Except that the layer forming conditions changed as shown in Table 25, the drums and the samples were made under the same fabrication apparatus and manner as Example 1 and were provided to examine the same items. The results are shown in Table 26. As the Table 26 illustrates, much defects on various items were acknowledged compared to the case of Example 11.

#### EXAMPLE 12

A light receiving member for use in electrophotography having a light receiving layer disposed on an Al cylinder having a mirror grinded surface was prepared under the layer forming conditions shown in Table 27 using the fabrication apparatus shown in FIG. 24.

And, a sample having only a surface layer on the same kind Al cylinder, another sample having only a charge injection prohibition layer on the same kind Al cylinder and further sample having only an IR layer on the same kind Al cylinder respectively as in the above case were provided.

For the resulting light receiving member, it was set with the conventional electrophotographic copying machine, and electrophotographic characteristics such as initial electrification efficiency, residual voltage and appearance of a ghost were examined, then decrease in the electrification efficiency, deterioration on photosensitivity and increase of defective images after 1,500 thousand times repeated shots were respectively examined.

Further, the situation of an image flow on the drum under high temperature and high humidity atmosphere at 35° C. and 85% humidity was also examined.

Then, a middle part was cut off from the above drum and engaged in quantitative analysis by IMA to analize the content of the elements in the thicknesswise direction.

As for the resulting first sample having only the surface layer, upper part, middle part and lower part of its image forming part were cut off, and were engaged in quantitative analysis by the conventional organic element analyzer to analize the content of hydrogen atoms in each of the cut-off parts.

As for the resulting second sample having only the charge injection prohibition layer and the resulting third sample having only the IR layer, in the same way as the above sample, upper part, middle part and lower part were cut off for each sample, and were subjected to the measurement of diffraction patterns corresponding to Si (111) near 27° of the diffraction angle by the conventional X-ray diffractometer to examine the existence of crystallinity.

The results of the various evaluations, the results of the quantitative analysis of the content of the hydrogen atoms, and the situations of crystallinity for the samples are as shown in Table 28.

And, the element profiles in the thicknesswise direction of the boron atoms (B) and the oxygen atoms (O) for the charge injection inhibition layer add the element

profile of the germanium atoms (Ge) for the IR layer are shown in FIG. 28.

As Table 28 and FIG. 28 illustrate, considerable advantages on items of initial electrification efficiency, image flow, residual voltage, ghost, defective image, increase in the defective image, and interference fringe were acknowledged.

#### EXAMPLE 13 (CONTANING COMPARATIVE EXAMPLE 4)

Multiple drums and samples for analysis were provided under the same conditions as in FIG. 11, except the conditions for forming a surface layer were changed to those shown in Table 29.

As a result of subjecting these drums and samples to the same evaluations and analyses as in Example 11, the results shown in Table 30 were obtained.

#### EXAMPLE 14

With the layer forming conditions for a photoconductive layer changed to the figures of Table 31, multiple drums having a light receiving layer were provided under the same conditions as in Example 11. These drums were examined by the same procedures as in Example 11. The results are shown in Table 32.

#### EXAMPLE 15

The same procedures of Example 11 were repeated, except that the layer forming conditions for forming a charge injection inhibition layer were changed as shown in Table 33, to thereby prepare multiple drums and samples having only a charge injection inhibition layer.

These drums and samples were examined by the same procedures as in Example 11. The results are shown in Table 34.

#### EXAMPLE 16

The same procedures of Example 11 were repeated, except that the layer forming conditions for forming a charge injection inhibition layer were changed as shown in Table 35, to thereby prepare multiple drums and samples having only a charge injection inhibition layer.

These drums and samples were examined by the same procedures as in Example 11. The results are shown in Table 36.

#### EXAMPLE 17

The same procedures of Example 11 were repeated, except that the layer forming conditions for forming an IR layer were changed as shown in Table 37, to thereby prepare multiple drums and samples having only an IR layer.

The resulting drums were examined by the same procedures as in Example 11.

As for the resulting samples, upper part, middle part and lower part were cut off for each sample, and were subjected to the measurement of diffraction patterns corresponding to Si (111) near 27° of the diffraction angle by the conventional X-ray diffractometer to examine the existence of crystallinity.

The results are shown in Table 38.

#### EXAMPLE 18

The same procedures of Example 11 were repeated, except that the layer forming conditions for forming an IR layer were changed as shown in Table 39, to thereby

prepare multiple drums and samples having only an IR layer.

The resulting drums were examined by the same procedures as in Example 11.

As for the resulting samples, upper part, middle part and lower part were cut off for each sample, and were subjected to the measurement of diffraction patterns corresponding to Si (111) near 27° of the diffraction angle by the conventional X-ray diffractometer to examine the existence of crystallinity.

The results are shown in Table 40.

#### EXAMPLE 19

The same procedures of Example 11 were repeated, except that the layer forming conditions for forming an IR layer were changed as shown in Table 41, to thereby prepare multiple drums and samples having only an IR layer.

The resulting drums were examined by the same procedures as in Example 11.

As for the resulting samples, upper part, middle part and lower part were cut off for each sample, and were subjected to the measurement of diffraction patterns corresponding to Si (111) near 27° of the diffraction angle by the conventional X-ray diffractometer to examine the existence of crystallinity.

The results are shown in Table 42.

#### EXAMPLE 20

The same procedures of Example 11 were repeated, except that the layer forming conditions for forming an IR layer were changed as shown in Table 43, to thereby prepare multiple drums and samples having only an IR layer.

The resulting drums were examined by the same procedures as in Example 11.

As for the resulting samples, upper part, middle part and lower part were cut off for each sample, and were subjected to the measurement of diffraction patterns corresponding to Si (111) near 27° of the diffraction angle by the conventional X-ray diffractometer to examine the existence of crystallinity.

The results are shown in Table 44.

#### EXAMPLE 21

On the same kind Al cylinder as in Example 1, a contact layer was formed under the layer forming conditions shown in Table 45, and a light receiving layer was formed on the contact layer by the same procedures as Example 11. And a sample having only a contact layer was also provided.

The resulting drums were examined by the same procedures as in Example 11.

As for the resulting samples, a part thereof was cut off for each sample, and was subjected to the measurement of diffraction patterns corresponding to Si (111) near 27° of the diffraction angle by the conventional X-ray diffractometer to examine the existence of crystallinity.

The results are shown in Table 46.

#### EXAMPLE 22

On the same kind Al cylinder as in Example 1, a contact layer was formed under the layer forming conditions shown in Table 47, and a light receiving layer was formed on the contact layer by the same procedures as Example 11. And a sample having only a contact layer was also provided.

The resulting drums were examined by the same procedures as in Example 11.

As for the resulting samples, a part thereof was cut off for each sample, and was subjected to the measurement of diffraction patterns corresponding to Si (111) near 27° of the diffraction angle by the conventional X-ray diffractometer to examine the existence of crystallinity.

The results are shown in Table 46.

### EXAMPLE 23

The mirror grinded Al cylinders were supplied for further grinding process with the use of a cutting tool having various angles. With the cross section form of FIG. 25 and the cross section patterns, multiple cylinders were provided. These cylinders were set to the fabrication apparatus of FIG. 24 accordingly to prepare drums by the same procedures as in Example 11. The resulting drums were evaluated with the conventional

electrophotographic copying machine having digital exposure functions and using semiconductor laser of 780 nm wavelength.

The results are shown in Table 50.

### EXAMPLE 24

The mirror grinded Al cylinders were engaged in further surface treatment to form uneven shape composed of a plurality of fine dimples at the surface, and 10 multiple cylinders having a cross section form of FIG. 26 and of a cross section pattern of Table 51 were provided. These cylinders were set to the fabrication apparatus of FIG. 24 accordingly and used for the preparation of drums under the same layer forming conditions 15 of Example 11. The resulting drums are evaluated with the conventional electrophotographic copying machine having digital exposure functions and using semiconductor laser of 780 nm wavelength. The results are shown in Table 52.

TABLE 1

| Name of layer                     | Gas used and flow rate (SCCM)                             |          | Substrate temperature (°C.) | RF power (W) | Internal pressure (torr) | Layer thickness (μm) |
|-----------------------------------|-----------------------------------------------------------|----------|-----------------------------|--------------|--------------------------|----------------------|
| Charge injection inhibition layer | SiH <sub>4</sub>                                          | 150      | 350                         | 1500         | 0.5                      | 1                    |
|                                   | B <sub>2</sub> H <sub>6</sub> (against SiH <sub>4</sub> ) | 1000 ppm |                             |              |                          |                      |
|                                   | NO                                                        | 10       |                             |              |                          |                      |
|                                   | H <sub>2</sub>                                            | 500      |                             |              |                          |                      |
| Photoconductive layer             | SiH <sub>4</sub>                                          | 350      | 250                         | 300          | 0.4                      | 20                   |
|                                   | H <sub>2</sub>                                            | 350      |                             |              |                          |                      |
| Surface layer                     | SiH <sub>4</sub>                                          | 10       | 250                         | 200          | 0.45                     | 0.5                  |
|                                   | CH <sub>4</sub>                                           | 500      |                             |              |                          |                      |
|                                   | H <sub>2</sub>                                            | 500      |                             |              |                          |                      |

TABLE 2

| Initial electrification efficiency | Initial sensitivity | Image flow | Residual voltage | Ghost | Defective image | Deterioration of sensitivity | Increase of defective image | Hydrogen content (atomic %) | Crystallinity |
|------------------------------------|---------------------|------------|------------------|-------|-----------------|------------------------------|-----------------------------|-----------------------------|---------------|
| ◎                                  | ○                   | ◎          | ◎                | ◎     | ○               | ○                            | ○                           | 52                          | Yes           |
| ◎ Excellent                        |                     |            |                  |       |                 |                              |                             |                             |               |
| ○ Good                             |                     |            |                  |       |                 |                              |                             |                             |               |
| Δ Practically applicable           |                     |            |                  |       |                 |                              |                             |                             |               |
| × Poor                             |                     |            |                  |       |                 |                              |                             |                             |               |

TABLE 3

| Name of layer                     | Gas used and flow rate (SCCM)                             |          | Substrate temperature (°C.) | RF power (W) | Internal pressure (torr) | Layer thickness (μm) |
|-----------------------------------|-----------------------------------------------------------|----------|-----------------------------|--------------|--------------------------|----------------------|
| Charge injection inhibition layer | SiH <sub>4</sub>                                          | 150      | 350                         | 1500         | 0.5                      | 1                    |
|                                   | B <sub>2</sub> H <sub>6</sub> (against SiH <sub>4</sub> ) | 1000 ppm |                             |              |                          |                      |
|                                   | NO                                                        | 10       |                             |              |                          |                      |
|                                   | H <sub>2</sub>                                            | 500      |                             |              |                          |                      |
| Photoconductive layer             | SiH <sub>4</sub>                                          | 350      | 250                         | 300          | 0.4                      | 20                   |
|                                   | H <sub>2</sub>                                            | 350      |                             |              |                          |                      |
| Surface layer                     | SiH <sub>4</sub>                                          | 10       | 150                         | 100          | 0.7                      | 0.5                  |
|                                   | CH <sub>4</sub>                                           | 500      |                             |              |                          |                      |
|                                   | H <sub>2</sub>                                            | 1000     |                             |              |                          |                      |

TABLE 4

| Initial electrification efficiency | Initial sensitivity | Image flow | Residual voltage | Ghost | Defective image | Deterioration of sensitivity | Increase of defective image | Hydrogen content (atomic %) | Crystallinity |
|------------------------------------|---------------------|------------|------------------|-------|-----------------|------------------------------|-----------------------------|-----------------------------|---------------|
| ×                                  | ○                   | ○          | ×                | Δ     | ×               | ○                            | ×                           | 87                          | Yes           |
| ◎ Excellent                        |                     |            |                  |       |                 |                              |                             |                             |               |
| ○ Good                             |                     |            |                  |       |                 |                              |                             |                             |               |
| Δ Practically applicable           |                     |            |                  |       |                 |                              |                             |                             |               |
| × Poor                             |                     |            |                  |       |                 |                              |                             |                             |               |

TABLE 5

| Name of layer    | Gas used and flow rate (SCCM) |  | Substrate temperature (°C.) | RF power (W) | Internal pressure (torr) | Layer thickness (μm) |
|------------------|-------------------------------|--|-----------------------------|--------------|--------------------------|----------------------|
| Charge injection | SiH <sub>4</sub>              |  | 150                         | 350          | 1500                     | 0.5                  |

TABLE 5-continued

| Name of layer         | Gas used and flow rate (SCCM)                                        | Substrate temperature (°C.) | RF power (W) | Internal pressure (torr) | Layer thickness (μm) |
|-----------------------|----------------------------------------------------------------------|-----------------------------|--------------|--------------------------|----------------------|
| inhibition layer      | B <sub>2</sub> H <sub>6</sub> (against SiH <sub>4</sub> ) 1000 ppm→0 |                             |              |                          |                      |
|                       | NO 10→0                                                              |                             |              |                          |                      |
|                       | H <sub>2</sub> 500                                                   |                             |              |                          |                      |
| Photoconductive layer | SiH <sub>4</sub> 350                                                 | 250                         | 300          | 0.4                      | 20                   |
|                       | H <sub>2</sub> 350                                                   |                             |              |                          |                      |
| Surface layer         | SiH <sub>4</sub> 10                                                  | 250                         | 200          | 0.4                      | 0.5                  |
|                       | CH <sub>4</sub> 400                                                  |                             |              |                          |                      |
|                       | H <sub>2</sub> 300                                                   |                             |              |                          |                      |

TABLE 6

| Initial electrification efficiency | Initial sensitivity | Image flow | Residual voltage | Ghost | Defective image | Deterioration of sensitivity | Increase of defective image | Hydrogen content (atomic %) | Crystallinity |
|------------------------------------|---------------------|------------|------------------|-------|-----------------|------------------------------|-----------------------------|-----------------------------|---------------|
| ◎                                  | ○                   | ◎          | ◎                | ◎     | ◎               | ◎                            | ○                           | ◎                           | 43            |
| ◎ Excellent                        | ○ Good              |            |                  |       |                 |                              |                             |                             | Yes           |
| △ Practically applicable           |                     |            |                  |       |                 |                              |                             |                             |               |
| ✗ Poor                             |                     |            |                  |       |                 |                              |                             |                             |               |

TABLE 7

| Drum No.                    | 301                 |                     |                     | 302                 |                     |                     | 303                 |                     |                     | 304                 |                     |                     | 305                 |                     |  | Comparative Example 2 |
|-----------------------------|---------------------|---------------------|---------------------|---------------------|---------------------|---------------------|---------------------|---------------------|---------------------|---------------------|---------------------|---------------------|---------------------|---------------------|--|-----------------------|
| Flow rate (SCCM)            | SiH <sub>4</sub> 10 | SiH <sub>4</sub> 10 | SiH <sub>4</sub> 10 | SiH <sub>4</sub> 10 | SiH <sub>4</sub> 10 | SiH <sub>4</sub> 10 | SiH <sub>4</sub> 10 | SiH <sub>4</sub> 10 | SiH <sub>4</sub> 10 | SiH <sub>4</sub> 10 | SiH <sub>4</sub> 10 | SiH <sub>4</sub> 10 | SiH <sub>4</sub> 10 | SiH <sub>4</sub> 10 |  |                       |
|                             | CH <sub>4</sub> 500 | CH <sub>4</sub> 500 | CH <sub>4</sub> 500 | CH <sub>4</sub> 500 | CH <sub>4</sub> 500 | CH <sub>4</sub> 500 | CH <sub>4</sub> 500 | CH <sub>4</sub> 500 | CH <sub>4</sub> 500 | CH <sub>4</sub> 500 | CH <sub>4</sub> 500 | CH <sub>4</sub> 500 | CH <sub>4</sub> 500 | CH <sub>4</sub> 500 |  |                       |
|                             | H <sub>2</sub> 300  | H <sub>2</sub> 500  | H <sub>2</sub> 700  | H <sub>2</sub> 700  | H <sub>2</sub> 700  | H <sub>2</sub> 700  | H <sub>2</sub> 700  | H <sub>2</sub> 700  | H <sub>2</sub> 700  | H <sub>2</sub> 800  |                     |                     |                     |                     |  |                       |
| Substrate temperature (°C.) | 250                 | 250                 | 250                 |                     |                     |                     | 150                 |                     | 150                 |                     | 100                 |                     |                     |                     |  |                       |
| RF power (W)                | 200                 | 100                 | 200                 | 200                 | 100                 | 100                 | 100                 | 100                 | 100                 | 100                 | 150                 |                     |                     |                     |  |                       |
| Internal pressure (torr)    | 0.4                 | 0.45                | 0.48                | 0.48                | 0.48                | 0.48                | 0.48                | 0.48                | 0.48                | 0.48                | 0.65                |                     |                     |                     |  |                       |
| Layer thickness (μm)        | 0.5                 | 0.5                 | 0.5                 | 0.5                 | 0.5                 | 0.5                 | 0.5                 | 0.5                 | 0.5                 | 0.5                 |                     |                     |                     |                     |  |                       |

TABLE 8

| Drum No.              | Initial electrification efficiency | Initial sensitivity | Image flow | Residual voltage | Ghost | Defective image | Deterioration of sensitivity | Increase of defective image | Sample No.              | Hydrogen content (atomic %) |
|-----------------------|------------------------------------|---------------------|------------|------------------|-------|-----------------|------------------------------|-----------------------------|-------------------------|-----------------------------|
| 301                   | ◎                                  | ○                   | ○          | ◎                | ○     | ◎               | ○                            | ○                           | 301-1                   | 43                          |
| 302                   | ◎                                  | ○                   | ◎          | ◎                | ○     | ○               | ○                            | ○                           | 302-1                   | 59                          |
| 303                   | ○                                  | ○                   | ◎          | ○                | ○     | ○               | ○                            | ○                           | 303-1                   | 61                          |
| 304                   | ○                                  | ○                   | ◎          | ○                | ○     | ○               | ○                            | ○                           | 304-1                   | 66                          |
| 305                   | ○                                  | ○                   | ○          | ○                | ○     | ○               | ○                            | ○                           | 305-1                   | 68                          |
| Comparative Example 2 | ✗                                  | ○                   | ○          | ×                | △     | ✗               | ○                            | ✗                           | Comparative Example 2-1 | 85                          |

◎ Excellent  
○ Good  
△ Practically applicable  
✗ Poor

TABLE 9

| Drum No.                    | 401                  |                      | 402                                                               |                      | 403                                                               |                      | 404                  |                      | 405                  |                      | 406                  |  |
|-----------------------------|----------------------|----------------------|-------------------------------------------------------------------|----------------------|-------------------------------------------------------------------|----------------------|----------------------|----------------------|----------------------|----------------------|----------------------|--|
| Flow rate (SCCM)            | SiH <sub>4</sub> 350 | SiH <sub>4</sub> 200 | SiH <sub>4</sub> 350                                              | SiH <sub>4</sub> 350 | SiH <sub>4</sub> 350                                              | SiH <sub>4</sub> 350 | SiH <sub>4</sub> 350 | SiH <sub>4</sub> 350 | SiH <sub>4</sub> 200 | SiH <sub>4</sub> 100 | SiF <sub>4</sub> 300 |  |
|                             | NO 50                | H <sub>2</sub> 600   | H <sub>2</sub> 350                                                | Ar 350               | He 350                                                            |                      |                      |                      |                      |                      |                      |  |
|                             |                      |                      | B <sub>2</sub> H <sub>6</sub> 0.3 ppm (against SiH <sub>4</sub> ) |                      | B <sub>2</sub> H <sub>6</sub> 0.3 ppm (against SiH <sub>4</sub> ) |                      |                      |                      |                      |                      |                      |  |
| Substrate temperature (°C.) | 250                  | 250                  |                                                                   | 250                  |                                                                   | 250                  |                      | 250                  |                      | 250                  |                      |  |
| RF power (W)                | 200                  | 400                  | 300                                                               | 250                  | 300                                                               | 300                  | 300                  | 300                  | 400                  |                      |                      |  |
| Internal pressure (torr)    | 0.4                  | 0.42                 | 0.4                                                               | 0.4                  | 0.4                                                               | 0.4                  | 0.4                  | 0.4                  | 0.38                 |                      |                      |  |
| Layer thickness (μm)        | 20                   | 20                   | 20                                                                | 20                   | 20                                                                | 20                   | 20                   | 20                   | 20                   |                      |                      |  |

TABLE 10

| Drum No. | Initial electrification efficiency | Initial sensitivity | Image flow | Residual voltage | Ghost | Defective image | Deterioration of sensitivity | Increase of defective image |
|----------|------------------------------------|---------------------|------------|------------------|-------|-----------------|------------------------------|-----------------------------|
| 401      | ◎                                  | ○                   | ○          | ○                | ○     | ○               | ○                            | ○                           |
| 402      | ◎                                  | ○                   | ○          | ○                | ○     | ○               | ○                            | ○                           |
| 403      | ○                                  | ○                   | ○          | ○                | ○     | ○               | ○                            | ○                           |
| 404      | ◎                                  | ○                   | ○          | ○                | ○     | ○               | ○                            | ○                           |
| 405      | ○                                  | ○                   | ○          | ○                | ○     | ○               | ○                            | ○                           |
| 406      | ◎                                  | ○                   | ○          | ○                | ○     | ○               | ○                            | ○                           |

◎ Excellent

○ Good

△ Practically applicable

× Poor

TABLE 11

| Drum No.                   | 501                                                                                              | 502                                                                                             | 503                                                                               | 504                                                                                  | 505*                                                                                  | 506                                                                                              |
|----------------------------|--------------------------------------------------------------------------------------------------|-------------------------------------------------------------------------------------------------|-----------------------------------------------------------------------------------|--------------------------------------------------------------------------------------|---------------------------------------------------------------------------------------|--------------------------------------------------------------------------------------------------|
| Flow rate (SCCM)           | SiH <sub>4</sub> 150                                                                             | SiH <sub>4</sub> 150                                                                            | SiH <sub>4</sub> 150                                                              | SiH <sub>4</sub> 150                                                                 | SiH <sub>4</sub> 150                                                                  | SiH <sub>4</sub> 100<br>SiF <sub>4</sub> 50                                                      |
|                            | B <sub>2</sub> H <sub>6</sub> 500 ppm (against SiH <sub>4</sub> )<br>NO 10<br>H <sub>2</sub> 500 | B <sub>2</sub> H <sub>6</sub> 100 ppm (against SiH <sub>4</sub> )<br>NO 5<br>H <sub>2</sub> 700 | PH <sub>3</sub> 100 ppm (against SiH <sub>4</sub> )<br>NO 5<br>H <sub>2</sub> 700 | B <sub>2</sub> H <sub>6</sub> 500 ppm (against SiH <sub>4</sub> )<br>NO 10<br>Ar 500 | B <sub>2</sub> H <sub>6</sub> 1000 ppm (against SiH <sub>4</sub> )<br>NO 10<br>He 500 | B <sub>2</sub> H <sub>6</sub> 500 ppm (against SiH <sub>4</sub> )<br>NO 10<br>H <sub>2</sub> 500 |
| Substrate temperature (°C) | 350                                                                                              | 350                                                                                             | 350                                                                               | 350                                                                                  | 350                                                                                   | 350                                                                                              |
| RF power (W)               | 1200                                                                                             | 1200                                                                                            | 1200                                                                              | 1500                                                                                 | 1500                                                                                  | 1500                                                                                             |
| Internal pressure (torr)   | 0.5                                                                                              | 0.5                                                                                             | 0.5                                                                               | 0.5                                                                                  | 0.5                                                                                   | 0.5                                                                                              |
| Layer thickness (μm)       | 1                                                                                                | 1                                                                                               | 1                                                                                 | 1                                                                                    | 1                                                                                     | 0.8                                                                                              |

\*Only the conditions for the photoconductive layer are the same as in the case of the drum No. 405

TABLE 12

| Drum No. | Initial electrification efficiency | Initial sensitivity | Image flow | Residual voltage | Ghost | Defective image | Deterioration of sensitivity | Increase of defective image | Remarks             | Sample No. | Crystallinity |
|----------|------------------------------------|---------------------|------------|------------------|-------|-----------------|------------------------------|-----------------------------|---------------------|------------|---------------|
| 501      | ◎                                  | ○                   | ○          | ○                | ○     | ○               | ○                            | ○                           |                     | 501-1      | Yes           |
| 502      | ○                                  | ○                   | ○          | ○                | ○     | ○               | ○                            | ○                           |                     | 502-1      | Yes           |
| 503      | ○                                  | ○                   | ○          | ○                | ○     | ○               | ○                            | ○                           | (-) electrification | 503-1      | Yes           |
| 504      | ◎                                  | ○                   | ○          | ○                | ○     | ○               | ○                            | ○                           |                     | 504-1      | Yes           |
| 505      | ○                                  | ○                   | ○          | ○                | ○     | ○               | ○                            | ○                           |                     | 505-1      | Yes           |
| 506      | ◎                                  | ○                   | ○          | ○                | ○     | ○               | ○                            | ○                           |                     | 506-1      | Yes           |

◎ Excellent

○ Good

△ Practically applicable

× Poor

TABLE 13

| Flow rate (SCCM)           | Drum No.             |                                                                                                      |                      |                                                                                                     |                                       |                                           |
|----------------------------|----------------------|------------------------------------------------------------------------------------------------------|----------------------|-----------------------------------------------------------------------------------------------------|---------------------------------------|-------------------------------------------|
|                            | 601                  |                                                                                                      | 602                  |                                                                                                     | 603                                   |                                           |
|                            | SiH <sub>4</sub> 150 | B <sub>2</sub> H <sub>6</sub> 500 ppm→0 (against SiH <sub>4</sub> )<br>NO 10→0<br>H <sub>2</sub> 500 | SiH <sub>4</sub> 150 | B <sub>2</sub> H <sub>6</sub> 100 ppm→0 (against SiH <sub>4</sub> )<br>NO 5→0<br>H <sub>2</sub> 700 | SiH <sub>4</sub> PH <sub>3</sub> 150  | 100 ppm→0<br>NO 5→0<br>H <sub>2</sub> 700 |
| Substrate temperature (°C) | 350                  |                                                                                                      | 350                  |                                                                                                     | 350                                   |                                           |
| RF power (W)               | 1200                 | 0.5                                                                                                  |                      | 1200                                                                                                | 0.5                                   | 1200                                      |
| Internal pressure (torr)   |                      |                                                                                                      |                      |                                                                                                     |                                       | 0.5                                       |
| Layer thickness (μm)       | 1                    |                                                                                                      | 1                    |                                                                                                     | 1                                     |                                           |
| Drum No.                   |                      |                                                                                                      |                      |                                                                                                     |                                       |                                           |
| Flow rate (SCCM)           | 604                  |                                                                                                      | 605*                 |                                                                                                     | 606                                   |                                           |
|                            | SiH <sub>4</sub> 150 | B <sub>2</sub> H <sub>6</sub> 500 ppm→0 (against SiH <sub>4</sub> )<br>NO 10→0                       | SiH <sub>4</sub> 150 | B <sub>2</sub> H <sub>6</sub> 1000 ppm→0 (against SiH <sub>4</sub> )<br>NO 10→0                     | SiH <sub>4</sub> SiF <sub>4</sub> 100 | 50<br>500 ppm→0                           |

TABLE 13-continued

|                             | Ar   | 500 | He | 500  | H <sub>2</sub> | 500  |
|-----------------------------|------|-----|----|------|----------------|------|
| Substrate temperature (°C.) |      | 350 |    | 350  |                | 350  |
| RF power (W)                | 1500 |     |    | 1500 |                | 1500 |
| Internal pressure (torr)    | 0.5  |     |    | 0.5  |                | 0.5  |
| Layer thickness (μm)        | 1    |     |    | 1    |                | 0.8  |

Only the conditions for the photoconductive layer are the same as in the case of the drum No. 405

TABLE 14

| Drum No. | Initial electrification efficiency | Initial sensitivity | Image flow | Residual voltage | Ghost | Defective image | Deterioration of sensitivity | Increase of defective image | Sample No. | Crystallinity |
|----------|------------------------------------|---------------------|------------|------------------|-------|-----------------|------------------------------|-----------------------------|------------|---------------|
| 601      | ◎                                  | ○                   | ○          | ◎                | ○     | ○               | ○                            | ○                           | 601-1      | Yes           |
| 602      | ○                                  | ○                   | ○          | ○                | ○     | ○               | ○                            | ○                           | 602-1      | Yes           |
| 603      | ○                                  | ○                   | ○          | ○                | ○     | ○               | ○                            | ○                           | 603-1      | Yes           |
| 604      | ○                                  | ○                   | ○          | ○                | ○     | ○               | ○                            | ○                           | 604-1      | Yes           |
| 605      | ○                                  | ○                   | ○          | ○                | ○     | ○               | ○                            | ○                           | 605-1      | Yes           |
| 606      | ◎                                  | ○                   | ○          | ○                | ○     | ○               | ○                            | ○                           | 606-1      | Yes           |

◎ Excellent

○ Good

△ Practically applicable

✗ Poor

TABLE 15

|                             | Drum No.         |                |                 | 30               |
|-----------------------------|------------------|----------------|-----------------|------------------|
|                             | 701              |                | 702             |                  |
|                             | SiH <sub>4</sub> | H <sub>2</sub> | NH <sub>3</sub> |                  |
| Flow rate (SCCM)            | 50               | 600            | 500             | SiH <sub>4</sub> |
| Substrate temperature (°C.) | 350              | 350            | 350             | H <sub>2</sub>   |
| RF power (W)                | 1000             | 1000           | 1000            | NH <sub>3</sub>  |
| Internal pressure (torr)    | 0.6              | 0.6            | 0.6             | NO               |
| Layer thickness (μm)        | 0.1              | 0.1            | 0.1             | N <sub>2</sub>   |

TABLE 17

| 35                          | Drum No.         |                |                |
|-----------------------------|------------------|----------------|----------------|
|                             | 801              |                | 802            |
|                             | SiH <sub>4</sub> | H <sub>2</sub> | N <sub>2</sub> |
| Flow rate (SCCM)            | 50               | 500            | 500            |
| Substrate temperature (°C.) | 250              | 250            | 250            |
| RF power (W)                | 150              | 200            | 200            |
| Internal pressure (torr)    | 0.3              | 0.3            | 0.3            |
| Layer thickness (μm)        | 0.1              | 0.1            | 0.1            |

TABLE 16

| Drum No. | Initial electrification efficiency | Initial sensitivity | Image flow | Residual voltage | Ghost | Defective image | Deterioration of sensitivity | Increase of defective image | Sample No. | Crystallinity |
|----------|------------------------------------|---------------------|------------|------------------|-------|-----------------|------------------------------|-----------------------------|------------|---------------|
| 701      | ◎                                  | ○                   | ○          | ○                | ○     | ○               | ○                            | ○                           | 701-1      | Yes           |
| 702      | ○                                  | ○                   | ○          | ○                | ○     | ○               | ○                            | ○                           | 702-1      | Yes           |
| 703      | ○                                  | ○                   | ○          | ○                | ○     | ○               | ○                            | ○                           | 703-1      | Yes           |

◎ Excellent

○ Good

△ Practically applicable

✗ Poor

TABLE 18

| Drum No. | Initial electrification efficiency | Initial sensitivity | Image flow | Residual voltage | Ghost | Defective image | Deterioration of sensitivity | Increase of defective image |
|----------|------------------------------------|---------------------|------------|------------------|-------|-----------------|------------------------------|-----------------------------|
| 801      | ○                                  | ○                   | ○          | ○                | ○     | ○               | ○                            | ○                           |
| 802      | ○                                  | ○                   | ○          | ○                | ○     | ○               | ○                            | ○                           |
| 803      | ○                                  | ○                   | ○          | ○                | ○     | ○               | ○                            | ○                           |

◎ Excellent

○ Good

△ Practically applicable

✗ Poor

TABLE 19

|   | a<br>[ $\mu\text{m}$ ] | Drum No. |     |     |     |     |
|---|------------------------|----------|-----|-----|-----|-----|
|   |                        | 901      | 902 | 903 | 904 | 905 |
| a | 25                     | 50       | 50  | 12  | 12  |     |
| b | 0.8                    | 2.5      | 0.8 | 1.5 | 0.3 |     |

TABLE 21

|                        | Drum No. |      |      |      |      |
|------------------------|----------|------|------|------|------|
|                        | 1001     | 1002 | 1003 | 1004 | 1005 |
| a<br>[ $\mu\text{m}$ ] | 50       | 100  | 100  | 30   | 30   |
| b<br>[ $\mu\text{m}$ ] | 2        | 5    | 1.5  | 2.5  | 0.7  |

TABLE 20

| Sample No. | Initial electrification efficiency | Initial sensitivity | Image flow | Interference fringe | Residual voltage | Ghost | Defective image | Deterioration of sensitivity | Increase of defective image | Image resolving power |
|------------|------------------------------------|---------------------|------------|---------------------|------------------|-------|-----------------|------------------------------|-----------------------------|-----------------------|
| 901        | ◎                                  | ○                   | ◎          | △                   | ◎                | ◎     | ◎               | ○                            | ◎                           | ○                     |
| 902        | ◎                                  | ○                   | ◎          | ○                   | ◎                | ◎     | ○               | ○                            | ◎                           | △                     |
| 903        | ◎                                  | ○                   | ◎          | △                   | ◎                | ◎     | ○               | ○                            | ◎                           | △                     |
| 904        | ◎                                  | ○                   | ◎          | ○                   | ◎                | ◎     | ○               | ○                            | ○                           | ○                     |
| 905        | ◎                                  | ○                   | ◎          | △                   | ◎                | ◎     | ○               | ○                            | ○                           | △                     |

◎ . . . Excellent  
○ . . . Good  
△ . . . Practically applicable  
x . . . Poor

TABLE 22

| Sample No. | Initial electrification efficiency | Initial sensitivity | Image flow | Interference fringe | Residual voltage | Ghost | Defective image | Deterioration of sensitivity | Increase of defective image | Image resolving power |
|------------|------------------------------------|---------------------|------------|---------------------|------------------|-------|-----------------|------------------------------|-----------------------------|-----------------------|
| 1001       | ◎                                  | ○                   | ◎          | △-                  | ◎                | ◎     | ◎               | ○                            | ◎                           | △                     |
| 1002       | ◎                                  | ○                   | ◎          | ○                   | ○                | ◎     | ○               | ○                            | ○                           | △                     |
| 1003       | ◎                                  | ○                   | ◎          | △                   | ○                | ○     | ○               | ○                            | ○                           | △                     |
| 1004       | ◎                                  | ○                   | ◎          | ○                   | ○                | ○     | ○               | ○                            | ○                           | ○                     |
| 1005       | ◎                                  | ○                   | ◎          | △-○                 | ○                | ○     | ○               | ○                            | ○                           | △-○                   |

◎ . . . Excellent  
○ . . . Good  
x . . . Practically applicable  
△ . . . Poor

TABLE 23

| Name of layer                     | Gas used and flow rate (SCCM)                             |          | Substrate temperature (°C.) | RF power (W) | Internal pressure (torr) | Layer thickness (μm) |
|-----------------------------------|-----------------------------------------------------------|----------|-----------------------------|--------------|--------------------------|----------------------|
| IR layer                          | SiH <sub>4</sub>                                          | 150      | 350                         | 1500         | 0.3                      | 0.1                  |
|                                   | B <sub>2</sub> H <sub>6</sub> (against SiH <sub>4</sub> ) | 1000 ppm |                             |              |                          |                      |
|                                   | NO                                                        | 10       |                             |              |                          |                      |
|                                   | GeH <sub>4</sub>                                          | 50       |                             |              |                          |                      |
|                                   | H <sub>2</sub>                                            | 500      |                             |              |                          |                      |
|                                   | SiH <sub>4</sub>                                          | 150      |                             |              |                          |                      |
| Charge injection inhibition layer | B <sub>2</sub> H <sub>6</sub> (against SiH <sub>4</sub> ) | 1000 ppm | 350                         | 1500         | 0.5                      | 1                    |
|                                   | NO                                                        | 10       |                             |              |                          |                      |
|                                   | H <sub>2</sub>                                            | 500      |                             |              |                          |                      |
| Photoconductive layer             | SiH <sub>4</sub>                                          | 350      | 250                         | 300          | 0.4                      | 20                   |
|                                   | H <sub>2</sub>                                            | 350      |                             |              |                          |                      |
| Surface layer                     | SiH <sub>4</sub>                                          | 10       | 250                         | 200          | 0.45                     | 0.5                  |
|                                   | CH <sub>4</sub>                                           | 500      |                             |              |                          |                      |
|                                   | H <sub>2</sub>                                            | 500      |                             |              |                          |                      |

TABLE 24

| Initial electrification efficiency | Initial sensitivity | Image flow | Interference fringe | Residual voltage | Ghost    | Defective image | Deterioration of sensitivity | Increase of defective image | Hydrogen content (atomic %) | Crystallinity |
|------------------------------------|---------------------|------------|---------------------|------------------|----------|-----------------|------------------------------|-----------------------------|-----------------------------|---------------|
| ◎                                  | ○                   | ◎          | ○                   | ◎                | ◎        | ◎               | ○                            | ○                           | ◎ 52                        | Yes           |
| IR layer                           | IR layer            | IR layer   | IR layer            | IR layer         | IR layer | IR layer        | IR layer                     | IR layer                    | IR layer                    | IR layer      |

◎ . . . Excellent  
○ . . . Good  
△ . . . Practically applicable  
x . . . Poor

TABLE 25

| Name of layer | Gas used and flow rate (SCCM)                             |          | Substrate temperature (°C.) | RF power (W) | Internal pressure (torr) | Layer thickness (μm) |
|---------------|-----------------------------------------------------------|----------|-----------------------------|--------------|--------------------------|----------------------|
| IR layer      | SiH <sub>4</sub>                                          | 150      | 350                         | 1500         | 0.3                      | 0.1                  |
|               | B <sub>2</sub> H <sub>6</sub> (against SiH <sub>4</sub> ) | 1000 ppm |                             |              |                          |                      |
|               | NO                                                        | 10       |                             |              |                          |                      |

TABLE 25-continued

| Name of layer                     | Gas used and flow rate (SCCM) |                                      | Substrate temperature (°C.) | RF power (W) | Internal pressure (torr) | Layer thickness (μm) |
|-----------------------------------|-------------------------------|--------------------------------------|-----------------------------|--------------|--------------------------|----------------------|
| Charge injection inhibition layer | GeH <sub>4</sub>              | 50                                   | 350                         | 1500         | 0.5                      | 1                    |
|                                   | H <sub>2</sub>                | 500                                  |                             |              |                          |                      |
|                                   | SiH <sub>4</sub>              | 150                                  |                             |              |                          |                      |
|                                   | B <sub>2</sub> H <sub>6</sub> | (against SiH <sub>4</sub> ) 1000 ppm |                             |              |                          |                      |
|                                   | NO                            | 10                                   |                             |              |                          |                      |
|                                   | H <sub>2</sub>                | 500                                  |                             |              |                          |                      |
| Photoconductive layer             | SiH <sub>4</sub>              | 350                                  | 250                         | 300          | 0.4                      | 20                   |
|                                   | H <sub>2</sub>                | 350                                  |                             |              |                          |                      |
| Surface layer                     | SiH <sub>4</sub>              | 10                                   | 150                         | 100          | 0.7                      | 0.5                  |
|                                   | CH <sub>4</sub>               | 500                                  |                             |              |                          |                      |
|                                   | H <sub>2</sub>                | 1000                                 |                             |              |                          |                      |

TABLE 26

| Initial electrification efficiency | Initial sensitivity | Image flow | Interference fringe | Residual voltage | Ghost | Defective image | Deterioration of sensitivity | Increase of defective image | Crystallinity               |                                   |          |
|------------------------------------|---------------------|------------|---------------------|------------------|-------|-----------------|------------------------------|-----------------------------|-----------------------------|-----------------------------------|----------|
|                                    |                     |            |                     |                  |       |                 |                              |                             | Hydrogen content (atomic %) | Charge injection inhibition layer | IR layer |
| x                                  | Q                   | ○          | ○                   | x                | Δ     | x               | x                            | ○                           | x                           | 87                                | Yes      |
| ○ Excellent                        | ○ Good              | ○ Good     | ○ Good              | x Poor           |       |                 |                              |                             |                             |                                   |          |

TABLE 27

| Name of layer                     | Gas used and flow rate (SCCM) |                                      | Substrate temperature (°C.) | RF power (W) | Internal pressure (torr) | Layer thickness (μm) |
|-----------------------------------|-------------------------------|--------------------------------------|-----------------------------|--------------|--------------------------|----------------------|
| IR layer                          | SiH <sub>4</sub>              | 150                                  | 350                         | 1500         | 0.3                      | 0.1                  |
|                                   | B <sub>2</sub> H <sub>6</sub> | (against SiH <sub>4</sub> ) 1000 ppm |                             |              |                          |                      |
|                                   | NO                            | 10                                   |                             |              |                          |                      |
|                                   | GeH <sub>4</sub>              | 50—0                                 |                             |              |                          |                      |
|                                   | H <sub>2</sub>                | 500                                  |                             |              |                          |                      |
|                                   | SiH <sub>4</sub>              | 150                                  |                             |              |                          |                      |
| Charge injection inhibition layer | B <sub>2</sub> H <sub>6</sub> | (against SiH <sub>4</sub> ) 1000 ppm | 350                         | 1500         | 0.5                      | 1                    |
|                                   | NO                            | 10—0                                 |                             |              |                          |                      |
|                                   | H <sub>2</sub>                | 500                                  |                             |              |                          |                      |
| Photoconductive layer             | SiH <sub>4</sub>              | 350                                  | 250                         | 300          | 0.4                      | 20                   |
|                                   | H <sub>2</sub>                | 350                                  |                             |              |                          |                      |
| Surface layer                     | SiH <sub>4</sub>              | 10                                   | 250                         | 200          | 0.45                     | 0.5                  |
|                                   | CH <sub>4</sub>               | 400                                  |                             |              |                          |                      |
|                                   | H <sub>2</sub>                | 300                                  |                             |              |                          |                      |

TABLE 28

| Initial electrification efficiency | Initial sensitivity | Image flow | Interference fringe | Residual voltage | Ghost | Defective image | Deterioration of sensitivity | Increase of defective image | Crystallinity               |                                   |          |
|------------------------------------|---------------------|------------|---------------------|------------------|-------|-----------------|------------------------------|-----------------------------|-----------------------------|-----------------------------------|----------|
|                                    |                     |            |                     |                  |       |                 |                              |                             | Hydrogen content (atomic %) | Charge injection inhibition layer | IR layer |
| ○                                  | ○                   | ○          | ○                   | ○                | ○     | ○               | ○                            | ○                           | 43                          | Yes                               | Yes      |

○ Excellent  
○ Good  
Δ Practically applicable  
x Poor

TABLE 29

|                             | Drum No.                                                         |                                                                  |                                                                  |                                                                  |                                                                  | Comparative Example 4                                            |
|-----------------------------|------------------------------------------------------------------|------------------------------------------------------------------|------------------------------------------------------------------|------------------------------------------------------------------|------------------------------------------------------------------|------------------------------------------------------------------|
|                             | 1301                                                             | 1302                                                             | 1303                                                             | 1304                                                             | 1305                                                             |                                                                  |
| Flow rate (SCCM)            | SiH <sub>4</sub> 10<br>CH <sub>4</sub> 500<br>H <sub>2</sub> 300 | SiH <sub>4</sub> 10<br>CH <sub>4</sub> 500<br>H <sub>2</sub> 500 | SiH <sub>4</sub> 10<br>CH <sub>4</sub> 500<br>H <sub>2</sub> 700 | SiH <sub>4</sub> 10<br>CH <sub>4</sub> 500<br>H <sub>2</sub> 700 | SiH <sub>4</sub> 10<br>CH <sub>4</sub> 500<br>H <sub>2</sub> 700 | SiH <sub>4</sub> 10<br>CH <sub>4</sub> 500<br>H <sub>2</sub> 800 |
| Substrate temperature (°C.) | 250                                                              | 250                                                              | 250                                                              | 150                                                              | 150                                                              | 100                                                              |
| RF power (W)                | 200                                                              | 100                                                              | 200                                                              | 200                                                              | 100                                                              | 150                                                              |
| Internal pressure (torr)    | 0.4                                                              | 0.45                                                             | 0.48                                                             | 0.48                                                             | 0.48                                                             | 0.65                                                             |
| Layer thickness (μm)        | 0.5                                                              | 0.5                                                              | 0.5                                                              | 0.5                                                              | 0.5                                                              | 0.5                                                              |

TABLE 30

| Drum No.              | Initial electrification efficiency | Initial sensitivity | Image flow | Interference fringe | Residual voltage | Ghost | Defective image | Deterioration of sensitivity | Increase of defective image | Sample No.              | Hydrogen content (atomic %) |
|-----------------------|------------------------------------|---------------------|------------|---------------------|------------------|-------|-----------------|------------------------------|-----------------------------|-------------------------|-----------------------------|
| 1301                  | ◎                                  | ○                   | ○          | ○                   | ○                | ○     | ○               | ○                            | ○                           | 1301-1                  | 44                          |
| 1302                  | ◎                                  | ○                   | ◎          | ○                   | ○                | ○     | ○               | ○                            | ○                           | 1302-1                  | 58                          |
| 1303                  | ○                                  | ○                   | ◎          | ○                   | ○                | ○     | ○               | ○                            | ○                           | 1303-1                  | 60                          |
| 1304                  | ○                                  | ○                   | ◎          | ○                   | ○                | ○     | ○               | ○                            | ○                           | 1304-1                  | 65                          |
| 1305                  | ○                                  | ○                   | ◎          | ○                   | ○                | ○     | ○               | ○                            | ○                           | 1305-1                  | 68                          |
| Comparative Example 4 | x                                  | ○                   | ○          | ○                   | x                | △     | x               | ○                            | x                           | Comparative Example 4-1 | 85                          |

◎Excellent

○ Good

△ Practically applicable

x Poor

TABLE 31

|                             | Drum No.                      |                                            |                                                                                                                    |                                |                                                                                                        |                                                                    |
|-----------------------------|-------------------------------|--------------------------------------------|--------------------------------------------------------------------------------------------------------------------|--------------------------------|--------------------------------------------------------------------------------------------------------|--------------------------------------------------------------------|
|                             | 1401                          | 1402                                       | 1403                                                                                                               | 1404                           | 1405                                                                                                   | 1406                                                               |
| Flow rate (SCCM)            | SiH <sub>4</sub> 350<br>NO 50 | SiH <sub>4</sub> 200<br>H <sub>2</sub> 600 | SiH <sub>4</sub> 350<br>H <sub>2</sub> 350<br>B <sub>2</sub> H <sub>6</sub> 0.3 ppm<br>(against SiH <sub>4</sub> ) | SiH <sub>4</sub> 350<br>Ar 350 | SiH <sub>4</sub> 350<br>He 350<br>B <sub>2</sub> H <sub>6</sub> 0.3 ppm<br>(against SiH <sub>4</sub> ) | SiH <sub>4</sub> 200<br>SiF <sub>4</sub> 100<br>H <sub>2</sub> 300 |
| Substrate temperature (°C.) | 250                           | 250                                        | 250                                                                                                                | 250                            | 250                                                                                                    | 250                                                                |
| RF power (W)                | 200                           | 400                                        | 300                                                                                                                | 250                            | 300                                                                                                    | 400                                                                |
| Internal pressure (torr)    | 0.4                           | 0.42                                       | 0.4                                                                                                                | 0.4                            | 0.4                                                                                                    | 0.38                                                               |
| Layer thickness (μm)        | 20                            | 20                                         | 20                                                                                                                 | 20                             | 20                                                                                                     | 20                                                                 |

TABLE 32

| Drum No. | Initial electrification efficiency | Initial sensitivity | Image flow | Interference fringe | Residual voltage | Ghost | Defective image | Deterioration of sensitivity | Increase of defective image |
|----------|------------------------------------|---------------------|------------|---------------------|------------------|-------|-----------------|------------------------------|-----------------------------|
| 1401     | ◎                                  | ○                   | ○          | ○                   | ○                | ○     | ○               | ○                            | ○                           |
| 1402     | ◎                                  | ○                   | ○          | ○                   | ○                | ○     | ○               | ○                            | ○                           |
| 1403     | ○                                  | ○                   | ○          | ○                   | ○                | ○     | ○               | ○                            | ○                           |
| 1404     | ◎                                  | ○                   | ○          | ○                   | ○                | ○     | ○               | ○                            | ○                           |
| 1405     | ○                                  | ○                   | ○          | ○                   | ○                | ○     | ○               | ○                            | ○                           |
| 1406     | ◎                                  | ○                   | ○          | ○                   | ○                | ○     | ○               | ○                            | ○                           |

◎Excellent

○ Good

△ Practically applicable

x Poor

TABLE 33

|                             | Drum No.                                                                                                                    |                                                                                                      |                                                                                        |
|-----------------------------|-----------------------------------------------------------------------------------------------------------------------------|------------------------------------------------------------------------------------------------------|----------------------------------------------------------------------------------------|
|                             | 1501                                                                                                                        | 1502                                                                                                 | 1503                                                                                   |
| Flow rate (SCCM)            | SiH <sub>4</sub> 150<br>B <sub>2</sub> H <sub>6</sub> 500 ppm<br>(against SiH <sub>4</sub> )<br>NO 10<br>H <sub>2</sub> 500 | SiH <sub>4</sub> 150<br>B <sub>2</sub> H <sub>6</sub> 100 ppm<br>(against SiH <sub>4</sub> )<br>NO 5 | SiH <sub>4</sub> 150<br>PH <sub>3</sub> 100 ppm<br>(against SiH <sub>4</sub> )<br>NO 5 |
| Substrate temperature (°C.) | 350                                                                                                                         | 350                                                                                                  | 350                                                                                    |
| RF power (W)                | 1200                                                                                                                        | 1200                                                                                                 | 1200                                                                                   |
| Internal pressure (torr)    | 0.5                                                                                                                         | 0.5                                                                                                  | 0.5                                                                                    |
| Layer thickness (μm)        | 1                                                                                                                           | 1                                                                                                    | 1                                                                                      |

  

|                             | Drum No.                                                                                                        |                                                                                                                  |                                                                                                                                                    |
|-----------------------------|-----------------------------------------------------------------------------------------------------------------|------------------------------------------------------------------------------------------------------------------|----------------------------------------------------------------------------------------------------------------------------------------------------|
|                             | 1504                                                                                                            | 1505                                                                                                             | 1506                                                                                                                                               |
| Flow rate (SCCM)            | SiH <sub>4</sub> 150<br>B <sub>2</sub> H <sub>6</sub> 500 ppm<br>(against SiH <sub>4</sub> )<br>NO 10<br>Ar 500 | SiH <sub>4</sub> 150<br>B <sub>2</sub> H <sub>6</sub> 1000 ppm<br>(against SiH <sub>4</sub> )<br>NO 10<br>He 500 | SiH <sub>4</sub> 100<br>SiF <sub>4</sub> 50<br>B <sub>2</sub> H <sub>6</sub> 500 ppm<br>(against SiH <sub>4</sub> )<br>NO 10<br>H <sub>2</sub> 500 |
| Substrate temperature (°C.) | 350                                                                                                             | 350                                                                                                              | 350                                                                                                                                                |
| RF power (W)                | 1500                                                                                                            | 1500                                                                                                             | 1500                                                                                                                                               |
| Internal pressure           | 0.5                                                                                                             | 0.5                                                                                                              | 0.5                                                                                                                                                |

TABLE 33-continued

| (torr)<br>Layer thickness<br>( $\mu\text{m}$ ) | 1 | 1 | 0.8 |
|------------------------------------------------|---|---|-----|
|------------------------------------------------|---|---|-----|

## Remarks

The conditions for the formation of the photoconductive layer are the same as in the case of the drum No. 1405

TABLE 34

| Drum No. | Initial electrification efficiency | Initial sensitivity | Image flow | Interference fringe | Residual voltage | Ghost | Defective image | Deterioration of sensitivity | Increase of defective image | Remarks | Sample No. | Crystallinity |
|----------|------------------------------------|---------------------|------------|---------------------|------------------|-------|-----------------|------------------------------|-----------------------------|---------|------------|---------------|
| 1501     | ◎                                  | ○                   | ○          | ○                   | ○                | ○     | ○               | ○                            | ○                           | (-)     | 1501-1     | Yes           |
| 1502     | ○                                  | ○                   | ○          | ○                   | ○                | ○     | ○               | ○                            | ○                           |         | 1502-1     | Yes           |
| 1503     | ○                                  | ○                   | ○          | ○                   | ○                | ○     | ○               | ○                            | ○                           |         | 1503-1     | Yes           |
| 1504     | ◎                                  | ○                   | ○          | ○                   | ○                | ○     | ○               | ○                            | ○                           |         | 1504-1     | Yes           |
| 1505     | ○                                  | ○                   | ○          | ○                   | ○                | ○     | ○               | ○                            | ○                           |         | 1505-1     | Yes           |
| 1506     | ◎                                  | ○                   | ○          | ○                   | ○                | ○     | ○               | ○                            | ○                           |         | 1506-1     | Yes           |

TABLE 35

| Drum No.                    | 1601                                                                                                           | 1602                                                                 | 1603                                                   | 1604                                                                 | 1605                                                                  | 1606                                                                 |
|-----------------------------|----------------------------------------------------------------------------------------------------------------|----------------------------------------------------------------------|--------------------------------------------------------|----------------------------------------------------------------------|-----------------------------------------------------------------------|----------------------------------------------------------------------|
| Flow rate (SCCM)            | SiH <sub>4</sub> 150                                                                                           | SiH <sub>4</sub> 150                                                 | SiH <sub>4</sub> 150                                   | SiH <sub>4</sub> 150                                                 | SiH <sub>4</sub> 150                                                  | SiH <sub>4</sub> 100<br>SiF <sub>4</sub> 50                          |
|                             | B <sub>2</sub> H <sub>6</sub> 500 ppm<br>(against SiH <sub>4</sub> )                                           | B <sub>2</sub> H <sub>6</sub> 100 ppm<br>(against SiH <sub>4</sub> ) | PH <sub>3</sub> 100 ppm<br>(against SiH <sub>4</sub> ) | B <sub>2</sub> H <sub>6</sub> 500 ppm<br>(against SiH <sub>4</sub> ) | B <sub>2</sub> H <sub>6</sub> 1000 ppm<br>(against SiH <sub>4</sub> ) | B <sub>2</sub> H <sub>6</sub> 500 ppm<br>(against SiH <sub>4</sub> ) |
|                             | NO 10→0                                                                                                        | NO 5→0                                                               | NO 5→0                                                 | NO 10→0                                                              | NO 10→0                                                               | NO 10→0                                                              |
| Substrate temperature (°C.) | H <sub>2</sub> 500                                                                                             | H <sub>2</sub> 700                                                   | H <sub>2</sub> 700                                     | Ar 500                                                               | He 500                                                                | H <sub>2</sub> 500                                                   |
| RF power (W)                | 1200                                                                                                           | 1200                                                                 | 1200                                                   | 1500                                                                 | 1500                                                                  | 1500                                                                 |
| Internal pressure (torr)    | 0.5                                                                                                            | 0.5                                                                  | 0.5                                                    | 0.5                                                                  | 0.5                                                                   | 0.5                                                                  |
| Layer thickness (μm)        | 1                                                                                                              | 1                                                                    | 1                                                      | 1                                                                    | 1                                                                     | 0.8                                                                  |
| Remarks                     | The conditions for the formation of the photoconductive layer are the same as in the case of the drum No. 1405 |                                                                      |                                                        |                                                                      |                                                                       |                                                                      |

TABLE 36

| Drum No. | Initial electrification efficiency | Initial sensitivity | Image flow | Interference fringe | Residual voltage | Ghost | Defective image | Deterioration of sensitivity | Increase of defective image | Sample No. | Crystallinity |
|----------|------------------------------------|---------------------|------------|---------------------|------------------|-------|-----------------|------------------------------|-----------------------------|------------|---------------|
| 1601     | ◎                                  | ○                   | ○          | ○                   | ○                | ○     | ○               | ○                            | ○                           | 1601-1     | Yes           |
| 1602     | ○                                  | ○                   | ○          | ○                   | ○                | ○     | ○               | ○                            | ○                           | 1602-1     | Yes           |
| 1603     | ○                                  | ○                   | ○          | ○                   | ○                | ○     | ○               | ○                            | ○                           | 1603-1     | Yes           |
| 1604     | ◎                                  | ○                   | ○          | ○                   | ○                | ○     | ○               | ○                            | ○                           | 1604-1     | Yes           |
| 1605     | ○                                  | ○                   | ○          | ○                   | ○                | ○     | ○               | ○                            | ○                           | 1605-1     | Yes           |
| 1606     | ◎                                  | ○                   | ○          | ○                   | ○                | ○     | ○               | ○                            | ○                           | 1606-1     | Yes           |

◎ Excellent

○ Good

△ Practically applicable

✗ Poor

TABLE 37

| Drum No.                    | 1701                                                                  | 1702                                                                 | 1703                                                   | 1704                                                                 | 1705-1                                                                | 1705-2                                                                | 1706                                                                  |
|-----------------------------|-----------------------------------------------------------------------|----------------------------------------------------------------------|--------------------------------------------------------|----------------------------------------------------------------------|-----------------------------------------------------------------------|-----------------------------------------------------------------------|-----------------------------------------------------------------------|
| Flow rate (SCCM)            | SiH <sub>4</sub> 150                                                  | SiH <sub>4</sub> 150                                                 | SiH <sub>4</sub> 150                                   | SiH <sub>4</sub> 150                                                 | SiH <sub>4</sub> 150                                                  | SiH <sub>4</sub> 150                                                  | SiH <sub>4</sub> 100<br>SiF <sub>4</sub> 50                           |
|                             | B <sub>2</sub> H <sub>6</sub> 1000 ppm<br>(against SiH <sub>4</sub> ) | B <sub>2</sub> H <sub>6</sub> 500 ppm<br>(against SiH <sub>4</sub> ) | PH <sub>3</sub> 100 ppm<br>(against SiH <sub>4</sub> ) | B <sub>2</sub> H <sub>6</sub> 500 ppm<br>(against SiH <sub>4</sub> ) | B <sub>2</sub> H <sub>6</sub> 1000 ppm<br>(against SiH <sub>4</sub> ) | B <sub>2</sub> H <sub>6</sub> 1000 ppm<br>(against SiH <sub>4</sub> ) | B <sub>2</sub> H <sub>6</sub> 1000 ppm<br>(against SiH <sub>4</sub> ) |
|                             | NO 10                                                                 | NO 5                                                                 | NO 5                                                   | NO 10                                                                | NO 10                                                                 | NO 10                                                                 | NO 10                                                                 |
|                             | GeH <sub>4</sub> 30                                                   | GeH <sub>4</sub> 50                                                  | GeH <sub>4</sub> 70                                    | GeH <sub>4</sub> 10                                                  | GeH <sub>4</sub> 50                                                   | GeH <sub>4</sub> 50                                                   | GeH <sub>4</sub> 50                                                   |
| Substrate temperature (°C.) | H <sub>2</sub> 500                                                    | H <sub>2</sub> 700                                                   | H <sub>2</sub> 700                                     | Ar 500                                                               | He 500                                                                | H <sub>2</sub> 500                                                    | H <sub>2</sub> 500                                                    |
| RF power (W)                | 1200                                                                  | 1200                                                                 | 1200                                                   | 1500                                                                 | 1500                                                                  | 1500                                                                  | 1500                                                                  |
| Internal pressure           | 0.3                                                                   | 0.3                                                                  | 0.3                                                    | 0.3                                                                  | 0.3                                                                   | 0.3                                                                   | 0.3                                                                   |

TABLE 37-continued

| Drum No.             | 1701 | 1702 | 1703 | 1704 | 1705-1 | 1705-2 | 1706 |
|----------------------|------|------|------|------|--------|--------|------|
| (torr)               |      |      |      |      |        |        |      |
| Layer thickness (μm) | 0.1  | 0.1  | 0.1  | 0.1  | 0.1    | 0.1    | 0.1  |
| Remarks              |      |      |      | *    | **     |        |      |

\*The conditions for the formation of the photoconductive layer are the same as in the case of the drum No. 1405. The conditions for the formation of the charge injection inhibition layer are the same as in the case of the drum No. 1505.

\*\*The conditions for the formation of the photoconductive layer are the same as in the case of the drum No. 1405. The conditions for the formation of the charge injection inhibition layer are the same as in the case of the drum No. 1605.

TABLE 38

| Drum No. | Initial electrification efficiency | Initial sensitivity | Image flow | Interference fringe | Residual voltage | Ghost | Defective image | Deterioration of sensitivity | Increase of defective image | Sample No. | Crystallinity |
|----------|------------------------------------|---------------------|------------|---------------------|------------------|-------|-----------------|------------------------------|-----------------------------|------------|---------------|
| 1701     | ○                                  | ○                   | ○          | ○                   | ○                | ○     | ○               | ○                            | ○                           | 1701-1     | Yes           |
| 1702     | ○                                  | ○                   | ○          | ○                   | ○                | ○     | ○               | ○                            | ○                           | 1702-1     | Yes           |
| 1703     | ○                                  | ○                   | ○          | ○                   | ○                | ○     | ○               | ○                            | ○                           | 1703-1     | Yes           |
| 1704     | ○                                  | ○                   | ○          | ○                   | ○                | ○     | ○               | ○                            | ○                           | 1704-1     | Yes           |
| 1705-1   | ○                                  | ○                   | ○          | ○                   | ○                | ○     | ○               | ○                            | ○                           | 1705-3     | Yes           |
| 1705-2   | ○                                  | ○                   | ○          | ○                   | ○                | ○     | ○               | ○                            | ○                           | 1705-4     | Yes           |
| 1706     | ○                                  | ○                   | ○          | ○                   | ○                | ○     | ○               | ○                            | ○                           | 1706-1     | Yes           |

○ Excellent

○ Good

Δ Practically applicable

✗ Poor

TABLE 39

| Drum No.                    | 1801                                                                  |     | 1802                                                                 |     | 1803                                                   |     | 1804                                                                 |     | 1805-1                                                                |     | 1805-2                                                                |     | 1806                                        |
|-----------------------------|-----------------------------------------------------------------------|-----|----------------------------------------------------------------------|-----|--------------------------------------------------------|-----|----------------------------------------------------------------------|-----|-----------------------------------------------------------------------|-----|-----------------------------------------------------------------------|-----|---------------------------------------------|
| Flow rate (SCCM)            | SiH <sub>4</sub>                                                      | 150 | SiH <sub>4</sub>                                                     | 150 | SiH <sub>4</sub>                                       | 150 | SiH <sub>4</sub>                                                     | 150 | SiH <sub>4</sub>                                                      | 150 | SiH <sub>4</sub>                                                      | 150 | SiH <sub>4</sub> 100<br>SiF <sub>4</sub> 50 |
|                             | B <sub>2</sub> H <sub>6</sub> 1000 ppm<br>(against SiH <sub>4</sub> ) |     | B <sub>2</sub> H <sub>6</sub> 500 ppm<br>(against SiH <sub>4</sub> ) |     | PH <sub>3</sub> 100 ppm<br>(against SiH <sub>4</sub> ) |     | B <sub>2</sub> H <sub>6</sub> 500 ppm<br>(against SiH <sub>4</sub> ) |     | B <sub>2</sub> H <sub>6</sub> 1000 ppm<br>(against SiH <sub>4</sub> ) |     | B <sub>2</sub> H <sub>6</sub> 1000 ppm<br>(against SiH <sub>4</sub> ) |     |                                             |
|                             | NO 10                                                                 |     | NO 5                                                                 |     | NO 5                                                   |     | NO 10                                                                |     | NO 10                                                                 |     | NO 10                                                                 |     |                                             |
|                             | GeH <sub>4</sub> 30→0<br>H <sub>2</sub> 500                           |     | GeH <sub>4</sub> 50→0<br>H <sub>2</sub> 700                          |     | GeH <sub>4</sub> 70→0<br>H <sub>2</sub> 700            |     | GeH <sub>4</sub> 10→0<br>Ar 500                                      |     | GeH <sub>4</sub> 50→0<br>He 500                                       |     | GeH <sub>4</sub> 50→0<br>H <sub>2</sub> 500                           |     |                                             |
| Substrate temperature (°C.) | 350                                                                   |     | 350                                                                  |     | 350                                                    |     | 350                                                                  |     | 350                                                                   |     | 350                                                                   |     | 350                                         |
| RF power (W)                | 1200<br>0.3                                                           |     | 1200<br>0.3                                                          |     | 1200<br>0.3                                            |     | 1500<br>0.3                                                          |     | 1500<br>0.3                                                           |     | 1500<br>0.3                                                           |     |                                             |
| Internal pressure (torr)    |                                                                       |     |                                                                      |     |                                                        |     |                                                                      |     |                                                                       |     |                                                                       |     |                                             |
| Layer thickness (μm)        | 0.1                                                                   |     | 0.1                                                                  |     | 0.1                                                    |     | 0.1                                                                  |     | 0.1                                                                   |     | 0.1                                                                   |     |                                             |
| Remarks                     |                                                                       |     |                                                                      |     |                                                        |     |                                                                      |     | *                                                                     | **  |                                                                       |     |                                             |

\*The conditions for the formation of the photoconductive layer are the same as in the case of the drum No. 1405. The conditions for the formation of the charge injection inhibition layer are the same as in the case of the Drum No. 1505.

\*\*The conditions for the formation of the photoconductive layer are the same as in the case of the drum No. 1405. The conditions for the formation of the charge injection inhibition layer are the same as in the case of the drum No. 1605.

TABLE 40

| Drum No. | Initial electrification efficiency | Initial sensitivity | Image flow | Interference fringe | Residual voltage | Ghost | Defective image | Deterioration of sensitivity | Increase of defective image | Sample No. | Crystallinity |
|----------|------------------------------------|---------------------|------------|---------------------|------------------|-------|-----------------|------------------------------|-----------------------------|------------|---------------|
| 1801     | ○                                  | ○                   | ○          | ○                   | ○                | ○     | ○               | ○                            | ○                           | 1801-1     | Yes           |
| 1802     | ○                                  | ○                   | ○          | ○                   | ○                | ○     | ○               | ○                            | ○                           | 1802-1     | Yes           |
| 1803     | ○                                  | ○                   | ○          | ○                   | ○                | ○     | ○               | ○                            | ○                           | 1803-1     | Yes           |
| 1804     | ○                                  | ○                   | ○          | ○                   | ○                | ○     | ○               | ○                            | ○                           | 1804-1     | Yes           |
| 1805-1   | ○                                  | ○                   | ○          | ○                   | ○                | ○     | ○               | ○                            | ○                           | 1805-3     | Yes           |
| 1805-2   | ○                                  | ○                   | ○          | ○                   | ○                | ○     | ○               | ○                            | ○                           | 1805-4     | Yes           |
| 1806     | ○                                  | ○                   | ○          | ○                   | ○                | ○     | ○               | ○                            | ○                           | 1806-1     | Yes           |

○ Excellent

○ Good

Δ Practically applicable

✗ Poor

TABLE 41

| Drum No.         | 1901             |     | 1902             |     | 1903             |     | 1904             |     | 1905-1           |     | 1905-2           |     | 1906                                        |
|------------------|------------------|-----|------------------|-----|------------------|-----|------------------|-----|------------------|-----|------------------|-----|---------------------------------------------|
| Flow rate (SCCM) | SiH <sub>4</sub> | 150 | SiH <sub>4</sub> | 150 | SiH <sub>4</sub> | 150 | SiH <sub>4</sub> | 150 | SiH <sub>4</sub> | 150 | SiH <sub>4</sub> | 150 | SiH <sub>4</sub> 100<br>SiF <sub>4</sub> 50 |

TABLE 41-continued

| Drum No.                    | 1901                                                                  | 1902                                                                 | 1903                                                   | 1904                                                                 | 1905-1                                                                | 1905-2                                                                | 1906                |
|-----------------------------|-----------------------------------------------------------------------|----------------------------------------------------------------------|--------------------------------------------------------|----------------------------------------------------------------------|-----------------------------------------------------------------------|-----------------------------------------------------------------------|---------------------|
|                             | B <sub>2</sub> H <sub>6</sub> 1000 ppm<br>(against SiH <sub>4</sub> ) | B <sub>2</sub> H <sub>6</sub> 500 ppm<br>(against SiH <sub>4</sub> ) | PH <sub>3</sub> 100 ppm<br>(against SiH <sub>4</sub> ) | B <sub>2</sub> H <sub>6</sub> 500 ppm<br>(against SiH <sub>4</sub> ) | B <sub>2</sub> H <sub>6</sub> 1000 ppm<br>(against SiH <sub>4</sub> ) | B <sub>2</sub> H <sub>6</sub> 1000 ppm<br>(against SiH <sub>4</sub> ) |                     |
| NO                          | 10                                                                    | NO 5                                                                 | NO 5                                                   | NO 10                                                                | NO 10                                                                 | NO 10                                                                 | NO 10               |
| GeH <sub>4</sub>            | 30                                                                    | GeH <sub>4</sub> 50                                                  | GeH <sub>4</sub> 70                                    | GeH <sub>4</sub> 10                                                  | GeH <sub>4</sub> 50                                                   | GeH <sub>4</sub> 50                                                   | GeH <sub>4</sub> 50 |
| H <sub>2</sub>              | 350                                                                   | H <sub>2</sub> 350                                                   | H <sub>2</sub> 350                                     | Ar 350                                                               | He 350                                                                | H <sub>2</sub> 350                                                    | H <sub>2</sub> 350  |
| Substrate temperature (°C.) | 250                                                                   | 250                                                                  | 250                                                    | 250                                                                  | 250                                                                   | 250                                                                   | 250                 |
| RF power (W)                | 150                                                                   | 200                                                                  | 150                                                    | 150                                                                  | 150                                                                   | 150                                                                   | 150                 |
| Internal pressure (torr)    | 0.27                                                                  | 0.27                                                                 | 0.27                                                   | 0.27                                                                 | 0.27                                                                  | 0.27                                                                  | 0.27                |
| Layer thickness (μm)        | 0.5                                                                   | 0.5                                                                  | 0.5                                                    | 0.5                                                                  | 0.5                                                                   | 0.5                                                                   | 0.4                 |
| Remarks                     |                                                                       |                                                                      |                                                        |                                                                      | *                                                                     | **                                                                    |                     |

\*The conditions for the formation of the photoconductive layer are the same as in the case of the drum No. 1405. The conditions for the formation of the charge injection inhibition layer are the same as in the case of the drum No. 1505.

\*\*The conditions for the formation of the photoconductive layer are the same as in the case of the drum No. 1405. The conditions for the formation of the charge injection inhibition layer are the same as in the case of the drum No. 1605.

TABLE 42

| Drum No. | Initial electrification efficiency | Initial sensitivity | Image flow | Interference fringe | Residual voltage | Ghost | Defective image | Deterioration of sensitivity | Increase of defective image |            |               |
|----------|------------------------------------|---------------------|------------|---------------------|------------------|-------|-----------------|------------------------------|-----------------------------|------------|---------------|
|          |                                    |                     |            |                     |                  |       |                 |                              | Sample No.                  | Sample No. | Crystallinity |
| 1901     | ◎                                  | ○                   | ○          | ○                   | ○                | ○     | ○               | ○                            | ○                           | 1901-1     | No            |
| 1902     | ◎                                  | ○                   | ○          | ○                   | ○                | ○     | ○               | ○                            | ○                           | 1902-1     | No            |
| 1903     | ◎                                  | ○                   | ○          | ○                   | ○                | ○     | ○               | ○                            | ○                           | 903-1      | No            |
| 1904     | ○                                  | ○                   | ○          | ○                   | ○                | ○     | ○               | ○                            | ○                           | 1904-1     | No            |
| 1905-1   | ○                                  | ○                   | ○          | ○                   | ○                | ○     | ○               | ○                            | ○                           | 1905-3     | No            |
| 1905-2   | ○                                  | ○                   | ○          | ○                   | ○                | ○     | ○               | ○                            | ○                           | 1905-4     | No            |
| 1906     | ◎                                  | ○                   | ○          | ○                   | ○                | ○     | ○               | ○                            | ○                           | 1906-1     | No            |

◎... Excellent

○... Good

Δ... Practically applicable

✗... Poor

TABLE 43

| Drum No.                    | 2001                                                                                          | 2002                                                                                         | 2003                                                                           | 2004                                                                                         | 2005-1                                                                                        | 2005-2                                                                                        | 2006               |
|-----------------------------|-----------------------------------------------------------------------------------------------|----------------------------------------------------------------------------------------------|--------------------------------------------------------------------------------|----------------------------------------------------------------------------------------------|-----------------------------------------------------------------------------------------------|-----------------------------------------------------------------------------------------------|--------------------|
| Flow rate (SCCM)            | SiH <sub>4</sub> 150<br>B <sub>2</sub> H <sub>6</sub> 1000 ppm<br>(against SiH <sub>4</sub> ) | SiH <sub>4</sub> 150<br>B <sub>2</sub> H <sub>6</sub> 500 ppm<br>(against SiH <sub>4</sub> ) | SiH <sub>4</sub> 150<br>PH <sub>3</sub> 100 ppm<br>(against SiH <sub>4</sub> ) | SiH <sub>4</sub> 150<br>B <sub>2</sub> H <sub>6</sub> 500 ppm<br>(against SiH <sub>4</sub> ) | SiH <sub>4</sub> 150<br>B <sub>2</sub> H <sub>6</sub> 1000 ppm<br>(against SiH <sub>4</sub> ) | SiH <sub>4</sub> 150<br>B <sub>2</sub> H <sub>6</sub> 1000 ppm<br>(against SiH <sub>4</sub> ) |                    |
|                             | NO 10                                                                                         | NO 5                                                                                         | NO 5                                                                           | NO 10                                                                                        | NO 10                                                                                         | NO 10                                                                                         |                    |
|                             | GeH <sub>4</sub> 30 → 0                                                                       | GeH <sub>4</sub> 50 → 0                                                                      | GeH <sub>4</sub> 70 → 0                                                        | GeH <sub>4</sub> 10 → 0                                                                      | GeH <sub>4</sub> 50 → 0                                                                       | GeH <sub>4</sub> 50 → 0                                                                       |                    |
|                             | H <sub>2</sub> 350                                                                            | H <sub>2</sub> 350                                                                           | H <sub>2</sub> 350                                                             | Ar 350                                                                                       | He 350                                                                                        | He 350                                                                                        | H <sub>2</sub> 350 |
| Substrate temperature (°C.) | 250                                                                                           | 250                                                                                          | 250                                                                            | 250                                                                                          | 250                                                                                           | 250                                                                                           | 250                |
| RF power (W)                | 150                                                                                           | 200                                                                                          | 150                                                                            | 150                                                                                          | 150                                                                                           | 150                                                                                           | 150                |
| Internal pressure (torr)    | 0.27                                                                                          | 0.27                                                                                         | 0.27                                                                           | 0.27                                                                                         | 0.27                                                                                          | 0.27                                                                                          | 0.27               |
| Layer thickness (μm)        | 0.5                                                                                           | 0.5                                                                                          | 0.5                                                                            | 0.5                                                                                          | 0.5                                                                                           | 0.5                                                                                           | 0.4                |
| Remarks                     |                                                                                               |                                                                                              |                                                                                |                                                                                              | *                                                                                             | ***                                                                                           |                    |

\*The conditions for the formation of the photoconductive layer are the same as in the case of the drum No. 1405. The conditions for the formation of the charge injection inhibition layer are the same as in the case of the drum No. 1505.

\*\*The conditions for the formation of the photoconductive layer are the same as in the case of the drum No. 1405. The conditions for the formation of the charge injection inhibition layer are the same as in the case of the drum No. 1605.

TABLE 44

| Drum No. | Initial electrification efficiency | Initial sensitivity | Image flow | Interference fringe | Residual voltage | Ghost | Defective image | Deterioration of sensitivity | Increase of defective image |            |               |
|----------|------------------------------------|---------------------|------------|---------------------|------------------|-------|-----------------|------------------------------|-----------------------------|------------|---------------|
|          |                                    |                     |            |                     |                  |       |                 |                              | Sample No.                  | Sample No. | Crystallinity |
| 2001     | ◎                                  | ○                   | ○          | ○                   | ○                | ○     | ○               | ○                            | ○                           | 2001-1     | No            |
| 2002     | ◎                                  | ○                   | ○          | ○                   | ○                | ○     | ○               | ○                            | ○                           | 2002-1     | No            |
| 2003     | ○                                  | ○                   | ○          | ○                   | ○                | ○     | ○               | ○                            | ○                           | 2003-1     | No            |
| 2004     | ○                                  | ○                   | ○          | ○                   | ○                | ○     | ○               | ○                            | ○                           | 2004-1     | No            |
| 2005-1   | ○                                  | ○                   | ○          | ○                   | ○                | ○     | ○               | ○                            | ○                           | 2005-3     | No            |
| 2005-2   | ○                                  | ○                   | ○          | ○                   | ○                | ○     | ○               | ○                            | ○                           | 2005-4     | No            |

TABLE 44-continued

| Drum No. | Initial electrification efficiency | Initial sensitivity | Image flow | Interference fringe | Residual voltage | Ghost | Defective image | Deterioration of sensitivity | Increase of defective image | Sample No. | Crystallinity |
|----------|------------------------------------|---------------------|------------|---------------------|------------------|-------|-----------------|------------------------------|-----------------------------|------------|---------------|
| 2006     | ◎                                  | ○                   | ○          | ◎                   | ◎                | ○     | ○               | ○                            | ○                           | ◎ 2006-1   | No            |

◎ . . Excellent  
 ○ . . Good  
 △ . . Practically applicable  
 × . . Poor

TABLE 45

| Drum No.                    | 2101                                                             | 2102                                                | 2103                                                            |  |
|-----------------------------|------------------------------------------------------------------|-----------------------------------------------------|-----------------------------------------------------------------|--|
| Flow rate (SCCM)            | SiH <sub>4</sub> 50<br>H <sub>2</sub> 600<br>NH <sub>3</sub> 500 | SiH <sub>4</sub> 50<br>H <sub>2</sub> 600<br>NO 500 | SiH <sub>4</sub> 50<br>H <sub>2</sub> 600<br>N <sub>2</sub> 500 |  |
| Substrate temperature (°C.) | 350                                                              | 350                                                 | 350                                                             |  |
| RF power (W)                | 1000                                                             | 1000                                                | 1000                                                            |  |
| Internal pressure (torr)    | 0.6                                                              | 0.6                                                 | 0.5                                                             |  |
| Layer thickness (μm)        | 0.1                                                              | 0.1                                                 | 0.1                                                             |  |

15

TABLE 47-continued

| Drum No.                    | 2201 | 2202 | 2203 |
|-----------------------------|------|------|------|
| Substrate temperature (°C.) | 250  | 250  | 250  |
| RF power (W)                | 150  | 200  | 200  |
| Internal pressure (torr)    | 0.3  | 0.3  | 0.3  |
| Layer thickness (μm)        | 0.1  | 0.1  | 0.1  |

TABLE 48

| Drum No. | Initial electrification efficiency | Initial sensitivity | Image flow | Interference fringe | Residual voltage | Ghost | Defective image | Deterioration of sensitivity | Increase of defective image | Sample No. | Crystallinity |
|----------|------------------------------------|---------------------|------------|---------------------|------------------|-------|-----------------|------------------------------|-----------------------------|------------|---------------|
| 2201     | ◎                                  | ○                   | ○          | ○                   | ○                | ○     | ○               | ○                            | ○                           | ◎ 2201-1   | No            |
| 2202     | ◎                                  | ○                   | ○          | ○                   | ○                | ○     | ○               | ○                            | ○                           | ◎ 2202-1   | No            |
| 2203     | ◎                                  | ○                   | ○          | ○                   | ○                | ○     | ○               | ○                            | ○                           | ◎ 2203-1   | No            |

◎ Excellent  
 ○ Good  
 △ Practically applicable  
 × Poor

(μm)

TABLE 49

| Drum No. | 2301 | 2302 | 2303 | 2304 | 2305 |
|----------|------|------|------|------|------|
|----------|------|------|------|------|------|

TABLE 46

| Drum No. | Initial electrification efficiency | Initial sensitivity | Image flow | Interference fringe | Residual voltage | Ghost | Defective image | Deterioration of sensitivity | Increase of defective image | Sample No. | Crystallinity |
|----------|------------------------------------|---------------------|------------|---------------------|------------------|-------|-----------------|------------------------------|-----------------------------|------------|---------------|
| 2101     | ◎                                  | ○                   | ○          | ○                   | ○                | ○     | ○               | ○                            | ○                           | ◎ 2101-1   | Yes           |
| 2102     | ◎                                  | ○                   | ○          | ○                   | ○                | ○     | ○               | ○                            | ○                           | ◎ 2102-1   | Yes           |
| 2103     | ◎                                  | ○                   | ○          | ○                   | ○                | ○     | ○               | ○                            | ○                           | ◎ 2103-1   | Yes           |

◎ Excellent  
 ○ Good  
 △ Practically applicable  
 × Poor

| Drum No.         | 2201                                       | 2202                          | 2203                                      |
|------------------|--------------------------------------------|-------------------------------|-------------------------------------------|
| Flow rate (SCCM) | SiH <sub>4</sub> 50<br>NH <sub>3</sub> 500 | SiH <sub>4</sub> 50<br>NO 500 | SiH <sub>4</sub> 50<br>N <sub>2</sub> 500 |

| a [μm] | 25  | 50  | 50  | 12  | 12  |
|--------|-----|-----|-----|-----|-----|
| b [μm] | 0.8 | 2.5 | 0.8 | 1.5 | 0.3 |

TABLE 50

| Drum No. | Initial electrification efficiency | Initial sensitivity | Image flow | Interference fringe | Residual voltage | Ghost | Defective image | Deterioration of sensitivity | Increase of defective image | Image resolving power |
|----------|------------------------------------|---------------------|------------|---------------------|------------------|-------|-----------------|------------------------------|-----------------------------|-----------------------|
| 2301     | ◎                                  | ○                   | ○          | ○                   | ○                | ○     | ○               | ○                            | ○                           | ○ ○                   |
| 2302     | ◎                                  | ○                   | ○          | ○                   | ○                | ○     | ○               | ○                            | ○                           | ○ ○                   |
| 2303     | ◎                                  | ○                   | ○          | ○                   | ○                | ○     | ○               | ○                            | ○                           | ○ △                   |
| 2304     | ◎                                  | ○                   | ○          | ○                   | ○                | ○     | ○               | ○                            | ○                           | ○ ○                   |
| 2305     | ◎                                  | ○                   | ○          | ○                   | ○                | ○     | ○               | ○                            | ○                           | ○ △                   |

◎ . . Excellent  
 ○ . . Good  
 △ . . Practically applicable  
 × . . Poor

TABLE 51

| Drum No. | 2401 | 2402 | 2403 | 2404 | 2405 |
|----------|------|------|------|------|------|
| c [μm]   | 50   | 100  | 100  | 30   | 30   |
| d [μm]   | 2    | 5    | 1.5  | 2.5  | 0.7  |

TABLE 52

| No.  | Initial electrifi-<br>efficiency | Initial<br>tivity | flow | Inter-<br>fringe | image | Ghost | image | Deterio-<br>ration of<br>tivity | Increase<br>of<br>image | Image<br>resolv-<br>power |
|------|----------------------------------|-------------------|------|------------------|-------|-------|-------|---------------------------------|-------------------------|---------------------------|
| 2401 | ◎                                | ○                 | ○    | ○                | ○     | ○     | ○     | ○                               | ○                       | △                         |
| 2402 | ◎                                | ○                 | ○    | ○                | ○     | ○     | ○     | ○                               | ○                       | △                         |
| 2403 | ◎                                | ○                 | ○    | ○                | ○     | ○     | ○     | ○                               | ○                       | △                         |
| 2404 | ○                                | ○                 | ○    | ○                | ○     | ○     | ○     | ○                               | ○                       | ○                         |
| 2405 | ○                                | ○                 | ○    | ○                | ○     | ○     | ○     | ○                               | ○                       | ○                         |

◎... Excellent

○... Good

△... Practically applicable

X... Poor

What we claim is:

1. A light receiving member for use in electrophotography comprising a substrate for electrophotography and a light receiving layer constituted by a charge injection inhibition layer formed of a polycrystal material containing silicon atoms as the main constituent atoms and an element for controlling the conductivity which functions to prevent a charge from being injected from the side of the substrate, a photoconductive layer formed of an amorphous material containing silicon atoms as the main constituent atoms and a surface layer formed of an amorphous material containing silicon atoms, carbon atoms and hydrogen atoms, the amount of the hydrogen atoms contained in the surface layer being in the range from 41 to 70 atomic %.

2. A light receiving member for use in electrophotography according to claim 1, wherein the charge injection inhibition layer contains the element for controlling the conductivity in the state of being distributed largely in the region adjacent to the substrate.

3. A light receiving member for use in electrophotography according to claim 1 or claim 2, wherein the charge injection prohibition layer contains at least one kind selected from nitrogen atoms, oxygen atoms and carbon atoms.

4. A light receiving member according to claim 2 wherein the charge injection inhibition layer contains at least one kind selected from nitrogen atoms, oxygen atoms and carbon atoms in the state of being distributed largely in the region adjacent to the substrate.

5. A light receiving member for use in electrophotography according to claim 1, wherein the photoconductive layer contains at least one kind selected from nitrogen atoms, oxygen atoms and an element for controlling the conductivity.

6. A light receiving member according to claim 1, wherein the element for controlling the conductivity is an element of the group III or V of the periodic table.

7. A light receiving member according to any of claim 1, wherein a contact layer formed of an amorphous material containing silicon atoms as the main constituent atoms, at least one kind selected from nitrogen atoms, oxygen atoms and carbon atoms, and in case where necessary, hydrogen atoms or/and halogen atoms is disposed between the substrate and the charge injection inhibition layer.

8. A light receiving member according to claim 1, wherein a contact layer formed of a polycrystal material containing silicon atoms as the main constituent atoms, at least one kind selected from nitrogen atoms,

oxygen atoms and carbon atoms, and in case where necessary, hydrogen atoms or/and halogen atoms is disposed between the substrate and the charge injection inhibition layer.

5 9. A light receiving member for use in electrophotography comprising a substrate for electrophotography

and a light receiving layer constituted by an absorption layer of light having a long wavelength (hereinafter referred to as "IR layer") formed of either a polycrystal material or an amorphous material containing silicon atoms and germanium atoms, a charge injection inhibition layer formed of a polycrystal material containing silicon atoms as the main constituent atoms and an element for controlling the conductivity which functions to prevent a charge from being injected from the side of the substrate, a photoconductive layer formed of an amorphous material containing silicon atoms as the main constituent atoms and a surface layer formed of an amorphous material containing silicon atoms, carbon atoms and hydrogen atoms, the amount of the hydrogen atoms contained in the surface layer being in the range from 41 to 70 atomic %.

10. A light receiving member for use in electrophotography according to claim 9, wherein the charge injection inhibition layer contains the element for controlling the conductivity in the state of being distributed largely in the region adjacent to the substrate.

11. A light receiving member for use in electrophotography according to claim 9 or claim 10, wherein the charge injection prohibition layer contains at least one kind selected from nitrogen atoms, oxygen atoms and carbon atoms.

12. A light receiving member according to claim 10, wherein the charge injection inhibition layer contains at least one kind selected from nitrogen atoms, oxygen atoms and carbon atoms in the state of being distributed largely in the region adjacent to the substrate.

13. A light receiving member for use in electrophotography according to claim 9, wherein the photoconductive layer contains at least one kind selected from nitrogen atoms, oxygen atoms and an element for controlling the conductivity.

14. A light receiving member for use in electrophotography according to claim 9, wherein the IR layer contains at least one kind selected from an element for controlling the conductivity, oxygen atoms, nitrogen atoms and carbon atoms.

15. A light receiving member according to claim 9, wherein the element for controlling the conductivity is an element of the group III or V of the periodic table.

16. A light receiving member according to claims 9, wherein the light receiving layer has a contact layer formed of an amorphous material containing silicon atoms as the main constituent atoms, at least one kind

selected from nitrogen atoms, oxygen atoms and carbon atoms, and in case where necessary, hydrogen atoms or/and halogen atoms.

17. A light receiving member according to claim 9, wherein the light receiving layer has a contact layer 5 formed of a polycrystal material containing silicon

atoms as the main constituent atoms, at least one kind selected from nitrogen atoms, oxygen atoms and carbon atoms, and in case where necessary, hydrogen atoms or/and halogen atoms.

\* \* \* \* \*

10

15

20

25

30

35

40

45

50

55

60

65

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL. Page 1 of 18

It is certified that error appears in the above-identified patent and that said Letters Patent is hereby corrected as shown below:

On the title page:

IN [75] INVENTORS

"Shigeru Shirai, Shiga;" should read  
--Shigeru Shirai, Nagahama;--.

COLUMN 1

Line 9, "those lights" should read --light--.  
Line 36, "mebbers" should read --members--.  
Line 46, "thecase" should read --the case--.

COLUMN 2

Line 15, "much" should read --very--.  
Line 19, "In consequence," should read  
--Consequently,--.  
Line 47, "structral" should read --structural--.  
Line 50, "frr" should read --for--.  
Line 65, "and quality." should read --and of high  
quality.--.  
Line 66, "Other" should read --Another--.

COLUMN 3

Line 8, "forcusing" should read --focusing--.  
Line 19, "abovementioned" should read --above-  
mentioned--.  
Line 36, "is ranging" should read --ranges--.

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL.

Page 2 of 18

It is certified that error appears in the above-identified patent and that said Letters Patent is hereby corrected as shown below:

COLUMN 4

Line 16, "along" should read --a long--.  
Line 17, "resistant" should read --resistant--.  
Line 25, "and quality" should read --and of  
high quality--.

COLUMN 6

Line 21, "strentth" should read --strength--.  
Line 31, "bite." should read --bit--.  
Line 39, "sirably" should read --sirable--.  
Line 49, "th" should read --the--.  
Line 64, "properl" should read --properly--.

COLUMN 7

Line 2, "surfcce" should read --surface--.  
Line 3, "dimention" should read --dimensions--.  
Line 34, "In alternative," should read  
--Alternatively,--.

COLUMN 8

Line 14, "graviationally" should read  
--gravitationally--.  
Line 20, "fur" should read --for--.

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL. Page 3 of 18

It is certified that error appears in the above-identified patent and that said Letters Patent is hereby corrected as shown below:

COLUMN 9

Line 35, "% more" should read --%, more--.

COLUMN 10

Line 26, "is no" should read --is in no--.

Line 39, "continuously" should read --continuously--.

Line 52, "ously" should read --ously--.

COLUMN 11

Line 7, "concentration (C" should read  
--concentration (C)--.

COLUMN 12

Line 1, "atom" should read --atoms--.

Line 6, "hydrogen atoms (X)" should read --halogen  
atoms (X)--.

Line 18, "referrig to FIGS. 8 12." should read  
--referring to FIGS. 8 through 12--.

Line 20, "gooup III" should read --group III--.

Line 58, "position t<sub>b</sub>" should read --position t<sub>b</sub>--.

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL. Page 4 of 18

It is certified that error appears in the above-identified patent and that said Letters Patent is hereby corrected as shown below:

COLUMN 13

Line 26, "represenss" should read --represents--.  
Line 27, "add" should read --and--.  
Line 31, "aayer" should read --layer--.  
Line 51, "distiibution" should read --distribution--.  
Line 55, "grddually" should read --gradually--.  
Line 56, "yously" should read --uously--.  
Line 61, "continyously" should read --continuously--.  
Line 66, "atims," should read --atoms,--.

COLUMN 15

Line 5, "or" should read --of--.  
Line 42, "5X10<sup>-4</sup>to" should read --5X10<sup>-4</sup> to--.  
Line 43, "1X10<sup>2</sup>to" should read --1X10<sup>2</sup> to--.  
Line 53, "chlorine and" should read --chlorine are--.

COLUMN 16

Line 29, "structually" should read --structurally--.  
Line 34, "in photoconductiveness" should read  
--nonphotoconductivity--.

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL.

Page 5 of 18

It is certified that error appears in the above-identified patent and that said Letters Patent is hereby corrected as shown below:

COLUMN 17

Line 8, "to" should be deleted.  
Line 11, "that" should read --it--.  
Line 15, "undesiable" should read --undesirable--.  
Line 17, "becasue os" should read --because of--.  
Line 35, "prbbles" should read --problems--.  
Line 48, "along" should read --a long--.  
Line 52, "above-mentione" should read --above-  
mentioned--.  
Line 54, "incorporttion" should read --incorporation--.  
Line 66, "rcceiv-" should read --receiv- --.

COLUMN 18

Line 3, "halongen" should read --halogen--.  
Line 29, "hhe" should read --the--.  
Line 63, "silico" should read --silicon--.

COLUMN 19

Line 4, "procsss," should read --process,--.  
Line 65, "aal" should read --ial--.

COLUMN 20

Line 26, "composed" should be deleted.

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL. Page 6 of 18

It is certified that error appears in the above-identified patent and that said Letters Patent is hereby corrected as shown below:

COLUMN 21

Line 7, "roducung" should read --producing--.  
Line 37, "contann" should read --contain--.  
Line 45, "constiuent" should read --constituent--.

COLUMN 22

Line 31, "nitoogen" should read --nitrogen--.

COLUMN 23

Line 46, "to as" should read --as--.  
Line 54, "aapable" should read --capable--.  
Line 63, "proeerties" should read --properties--.

COLUMN 24

Line 34, "1X10 to 1 Torr;" should read  
-- $1 \times 10^{-1}$  to 1 Torr;--.  
Line 55, "flow" should read --glow-- and  
"orion" should read --or ion--.  
Line 65, "in on" should read --in an--.  
Line 67, "(si<sub>x</sub>C<sub>1-x</sub>)<sub>y</sub>:" should read --(Si<sub>x</sub>C<sub>1-x</sub>)<sub>y</sub>:--.

COLUMN 26

Line 2, "wihh" should read --with--.  
Line 34, "frm" should read --from--.

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL.

Page 7 of 18

It is certified that error appears in the above-identified patent and that said Letters Patent is hereby corrected as shown below:

COLUMN 27

Line 6, "vacuum" should read --vacuum gauge--.  
Line 18, "412," should read --2412,--.  
Line 26, "CH<sub>4</sub>" should read --H<sub>2</sub>--.  
Line 31, "the 2437" should read --the substrate cylinder 2437--.  
Line 31, "heater 2448" should read --heater 2438--.  
Lines 45-48, Italics should be deleted.  
Line 51, "atoms in" should read --atoms is--.  
Line 52, "in stead" should read --instead--.  
Line 61, "wher" should read --where--.  
Line 63, "in stead" should read --instead--.  
Line 64, "holds" should read --folds--.  
Line 65, "rised." should read --raised.--.

COLUMN 28

Line 16, "upon" should be deleted.  
Line 29, "cllinder" should read --cylinder--.  
Line 35, "werepre-" should read --were pre- --.

COLUMN 29

Line 38, "flow or" should read --flow on--.

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL. Page 8 of 18

It is certified that error appears in the above-identified patent and that said Letters Patent is hereby corrected as shown below:

COLUMN 30

Line 25, "conditios" should read --conditions--.  
Lines 27-28, "Table 12. ¶ With" should read  
--Table 12. ¶ EXAMPLE 6 ¶ With--.  
Line 44, "in the" should read --using the--.  
Line 45, "there" should read --they--.

COLUMN 31

Line 20, "are" should read --were--.  
Line 30, "Table 33" should read --Table 23--.  
Line 55, "iddle" should read --middle--.  
Line 60, "Asffor" should read --As for--.

COLUMN 32

Line 28, "aame" should read --same--.  
Line 32, "suhh" should read --such--.  
Line 68, "add" should read --and--.

COLUMN 33

Line 12, "FIG. 11," should read --Example 11,--.  
Line 55, "bytthe" should read --by the--.

COLUMN 36

Line 16, "oopying" should read --copying--.

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL. Page 9 of 18

It is certified that error appears in the above-identified patent and that said Letters Patent is hereby corrected as shown below:

COLUMN 39

TABLE 12, "flow      voltage      Ghost      image

| flow | voltage | Ghost | image |
|------|---------|-------|-------|
| ○    | ○       | ○     | ○     |
| ○    | ○       | ○     | ○     |
| ○    | ○       | ○     | ○     |
| ○    | ○       | ○     | ○     |
| ○    | ○       | ○     | ○     |
| ○    | ○       | ○     | ○     |
| ○    | ○       | ○     | ○     |
| ○    | ○       | ○     | ○     |

"

should read --flow      voltage      Ghost      image

| flow | voltage | Ghost | image |
|------|---------|-------|-------|
| ○    | ○       | ○     | ○     |
| ○    | ○       | ○     | ○     |
| ○    | ○       | ○     | ○     |
| ○    | ○       | ○     | ○     |
| ○    | ○       | ○     | ○     |
| ○    | ○       | ○     | ○     |
| ○    | ○       | ○     | ○     |
| ○    | ○       | ○     | ○     |

---

COLUMN 40

TABLE 13, "PH<sub>3</sub>      100 ppm→0      should --PH<sub>3</sub>      100 ppm→0

read      (against SiH<sub>4</sub>)

NO      5→0      "      NO      5→0      ---.

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL. Page 10 of 18

It is certified that error appears in the above-identified patent and that said Letters Patent is hereby corrected as shown below:

COLUMN 40

TABLE 13, "B<sub>2</sub>H<sub>6</sub> 500 ppm→0 should --B<sub>2</sub>H<sub>6</sub> 500 ppm→0  
read (against SiH<sub>4</sub>)  
NO 10→0 " NO 10→0 --.

COLUMN 41

TABLE 14, "Ghost  
◎  
◎  
◎  
◎  
◎  
◎ " should --Ghost  
read ◎  
◎  
◎  
◎  
◎  
◎ --.

COLUMN 41

TABLE 16, "Defective image " should --Defective image --.

COLUMN 42

TABLE 18, "Defective image " should --Defective image --.

COLUMN 43

TABLE 22, "fringe Δ- " should --fringe Δ- --.

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL. Page 11 of 18

It is certified that error appears in the above-identified patent and that said Letters Patent is hereby corrected as shown below:

COLUMNS 43-44

TABLE 24,

"flow  $\odot$  fringe  $\circ$  voltage  $\odot$  Ghost  $\odot$  image  $\circ$  sensitivitiy  $\odot$  image  $\odot$ "  
should read

--flow  $\odot$  fringe  $\circ$  voltage  $\odot$  Ghost  $\odot$  image  $\circ$  sensitivitiy  $\odot$  image  $\odot$  --.

COLUMN 45

TABLE 26, "O Excellent" should read -- $\odot$  Excellent--.  
TABLE 28, "O Excellent" should read -- $\odot$  Excellent--.

COLUMN 45

TABLE 28,

"flow  $\odot$  fringe  $\odot$  voltage  $\odot$  Ghost  $\odot$  image  $\circ$  sensitivitiy  $\odot$  "

should read

--flow  $\odot$  fringe  $\odot$  voltage  $\odot$  Ghost  $\odot$  image  $\circ$  sensitivitiy  $\odot$  --.

UNITED STATES PATENT AND TRADEMARK OFFICE  
**CERTIFICATE OF CORRECTION**

PATENT NO. : 4,792,509

DATED : December 20, 1988

INVENTOR(S) : SHIGERU SHIRAI, ET AL. Page 12 of 18

It is certified that error appears in the above-identified patent and that said Letters Patent is hereby corrected as shown below:

COLUMN 47

TABLE 30, " 1305   ○   ○ should   -- 1305   ○   ○  
 Compar-   x○"   read   Compar-   x   ○ --.

COLUMNS 49-50

TABLE 34, "voltage Ghost image sensitivity

should read --voltage Ghost image sensitivity

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL. Page 13 of 18

It is certified that error appears in the above-identified patent and that said Letters Patent is hereby corrected as shown below:

COLUMNS 49-50

TABLE 36, "voltage Ghost image sensitivity image

|   |   |   |   |   |   |
|---|---|---|---|---|---|
| ◎ | ◎ | ◎ | ◎ | ◎ | ◎ |
| ◎ | ◎ | ◎ | ◎ | ◎ | ◎ |
| ◎ | ◎ | ◎ | ◎ | ◎ | ◎ |
| ◎ | ◎ | ◎ | ◎ | ◎ | ◎ |
| ◎ | ◎ | ◎ | ◎ | ◎ | ◎ |
| ◎ | ◎ | ◎ | ◎ | ◎ | ◎ |
| ◎ | ○ | ○ | ○ | ○ | ○ |

should read

--voltage Ghost image sensitivity image

|   |   |   |   |   |    |
|---|---|---|---|---|----|
| ◎ | ◎ | ◎ | ○ | ◎ |    |
| ◎ | ◎ | ◎ | ○ | ◎ |    |
| ◎ | ◎ | ○ | ○ | ○ |    |
| ◎ | ◎ | ○ | ○ | ◎ |    |
| ◎ | ◎ | ◎ | ○ | ◎ |    |
| ◎ | ○ | ○ | ○ | ○ | -- |

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL. Page 14 of 18

It is certified that error appears in the above-identified patent and that said Letters Patent is hereby corrected as shown below:

COLUMN 51

TABLE 38,

|             |        |        |              |        |
|-------------|--------|--------|--------------|--------|
| "efficiency | tivity | should | --efficiency | tivity |
| ○           | ○      | read   | ○            | ○      |
| ○           | ○      |        | ○            | ○      |
| ○           | ○      |        | ○            | ○      |
| ○           | ○      |        | ○            | ○      |
| ○           | ○      | "      | ○            | ○      |
| ○           | ○      |        | ○            | ○      |
|             |        |        | ---          |        |

COLUMN 53

TABLE 42, "1905--1  
1905--2" should --1905-1  
read 1905-2--.

UNITED STATES PATENT AND TRADEMARK OFFICE  
**CERTIFICATE OF CORRECTION**

PATENT NO. : 4,792,509

DATED : December 20, 1988

INVENTOR(S) : SHIGERU SHIRAI, ET AL. Page 15 of 18

It is certified that error appears in the above-identified patent and that said Letters Patent is hereby corrected as shown below:

COLUMNS 53-54

TABLE 42.

should read

UNITED STATES PATENT AND TRADEMARK OFFICE  
**CERTIFICATE OF CORRECTION**

PATENT NO. : 4,792,509

DATED : December 20, 1988

INVENTOR(S) : SHIGERU SHIRAI, ET AL.

Page 16 of 18

It is certified that error appears in the above-identified patent and that said Letters Patent is hereby corrected as shown below:

**COLUMNS 53-54**

TABLE 44, "fringe voltage Ghost image sensitivity

A decorative horizontal border consisting of a repeating pattern of small circles and ovals, rendered in a light blue-grey color.

should read

--fringe voltage Ghost image sensitivity

A decorative border made of a repeating pattern of small circles, consisting of four vertical columns of circles.

— 2 —

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL. Page 17 of 18

It is certified that error appears in the above-identified patent and that said Letters Patent is hereby corrected as shown below:

COLUMNS 57-58

TABLE 52

|  | Initial<br>electrifi-<br>No. efficiency | Initial<br>tivity | Inter-<br>flow | fringe | image | Ghost |
|--|-----------------------------------------|-------------------|----------------|--------|-------|-------|
|--|-----------------------------------------|-------------------|----------------|--------|-------|-------|

(table continued below due to lack of space)

|                                |                          |                            |
|--------------------------------|--------------------------|----------------------------|
| Deterio-<br>ration of<br>image | Increase<br>of<br>tivity | Image<br>resolv-<br>power" |
|--------------------------------|--------------------------|----------------------------|

should read

| -- | Initial<br>electrifi-<br>Drum cation | Initial<br>sensi-<br>tivity | Inter-<br>Image<br>flow | ference<br>fringe | Residual<br>image | Ghost |
|----|--------------------------------------|-----------------------------|-------------------------|-------------------|-------------------|-------|
|----|--------------------------------------|-----------------------------|-------------------------|-------------------|-------------------|-------|

(table continued below due to lack of space)

|                    |                                           |                                      |                                      |
|--------------------|-------------------------------------------|--------------------------------------|--------------------------------------|
| Defection<br>image | Deterio-<br>ration of<br>sensi-<br>tivity | Increase<br>of<br>defective<br>image | Image<br>resolv-<br>ing<br>power --. |
|--------------------|-------------------------------------------|--------------------------------------|--------------------------------------|

UNITED STATES PATENT AND TRADEMARK OFFICE  
CERTIFICATE OF CORRECTION

PATENT NO. : 4,792,509

DATED : December 20, 1988

INVENTOR(S) : SHIGERU SHIRAI, ET AL. Page 18 of 18

It is certified that error appears in the above-identified patent and that said Letters Patent is hereby corrected as shown below:

COLUMN 57

Line 34, "mmember" should read --member--.  
Line 41, "prohibition" should read --inhibition--.  
Line 44, "claim 2" should read --claim 2,--.  
Line 57, "any of" should be deleted.

COLUMN 58

Line 44, "prohibition" should read --inhibition--.  
Line 65, "claims 9," should read --claim 9,--.

Signed and Sealed this

Twenty-seventh Day of March, 1990

*Attest:*

JEFFREY M. SAMUELS

*Attesting Officer*

*Acting Commissioner of Patents and Trademarks*